# EUROPEAN PATENT SPECIFICATION

(11) **EP 0 212 284 B1**
(45) Date of publication and mention of the grant of the patent: **22.09.1993**
(21) Application number: 86109998.4
(22) Date of filing: 21.07.1986
(51) Int. Cl.: D04H 1/56, D04H 13/00

(54) **Gathered nonwoven elastic web**
Nichtgewebtes elastisches Plissee
Etoffe non tissée élastique froncée

(30) Priority: 30.07.1985 US 760445; 30.07.1985 US 760449
(43) Date of publication of application: 04.03.1987
(73) Proprietor: KIMBERLY-CLARK CORPORATION, Neenah, Wisconsin 54956-0349 (US)
(72) Inventor: Morman, Michael Tod, Alpharetta Georgia (US)
(74) Representative: Grünecker, Kinkeldey, Stockmair & Schwanhäusser Anwaltssozietät

(56) References cited:
- WO-A-80/00676
- US-A- 2 957 512
- US-A- 4 100 324

## Description

The present invention relates to a process for forming a composite nonwoven elastic web which is joined to a nonwoven gathered web and to a process for forming a gathered nonwoven web exhibiting elastic properties when separated from the nonwoven elastic web after gathering has been effected by retraction of the elastic web.

There has been a desire in the area of diaper fabrication to provide an outer cover for a diaper which is (1) totally elastic over its entire surface --to provide a tight yet comfortable fit; (2) water repellent --to retain fluid materials within the confines of the diaper; (3) breathable --to allow an exchange of vapors through the diaper material; (4) soft --for improved comfort and (5) inexpensive to manufacture --so that that diaper may be economically marketed to the consumer.

Unfortunately, the known composite nonwoven materials which have, to date, been marketed have been lacking in one or more of these characteristics. Furthermore, these composite elastic nonwoven materials have not been formed by utilization of economical processes.

For example, U.S. patent 2,957,512 to Wade discloses a method for producing an elastic composite sheet material in which a creped or corrugated flexible sheet material is bonded to, for example, an elastic meltblown material. At column 5, lines 39-48, it is stated that a fibrous web of elastomeric material may be stretched and bonded to the corrugated web at spaced points or areas and, upon allowing the fibrous elastomeric web to relax, the composite will assume the structure illustrated in Figure 7.

Yet another method for forming a composite elastic fabric is disclosed in U.S. patent 3,316,136 to Pufahl. The preferred method of fabrication of this fabric involves the utilization of an adhesive which is first applied in a predetermined pattern to an elastic backing material and the elastic backing material is then stretched to an elongated state. While the elastic material is in the stretched, elongated state an overlying fabric is placed in contact therewith and held in pressurized engagement with the elastic material for a time period sufficient to insure adhesion of the two layers. Thereafter, upon drying of the applied adhesive, the tension on the elastic backing material is released causing the overlying fabric to gather in the areas outlined by the adhesive.

U.S. Patent 3,485,706 to Evans at example 56 discloses the fabrication of an elongatable nonwoven, multilevel patterned structure having elasticity in one direction from an initially layered material. The structure is composed of two webs of polyester staple fibers which have a web of spandex yarn located therebetween. The webs are joined to each other by application of hydraulic jets of water which entangle the fibers of one web with the fibers of an adjacent web. During the entanglement step the spandex yarn is stretched 200 percent.

U.S. Patent 3,673,026 to Brown discloses a method for manufacturing a laminated fabric and specifically discloses a method for manufacturing a nonwoven laminated fabric of controlled bulk. In this method separate webs of nonwoven material, e.g. creped tissue or bonded synthetic fiber, are elastically stretched to different degrees of elongation and laminated by bonding to one another while in their differentially stretched states. The bonded webs are thereafter relaxed so as to produce different degrees of contraction in each web with resultant separation of the webs in the unbonded regions and controlled bulk in the laminate. It is stated that the differential stretching includes the situation where only one web is actually stretched and the other web is maintained slack or nearly so.

U.S. patent 3,687,797 to Wideman discloses a method for producing a resilent cellulosic wadding product obtained by laminating a lower cellulosic wadding web to a prestretched polyurethane foam web. The process involves applying adhesive in a desired pattern to either of the webs with the wadding web then being laminated to the prestretched polyurethane foam web. During lamination of the wadding web to the polyurethane foam web the foam web is maintained in a stretched condition. After lamination of the two webs, the tension on the prestretched polyurethane foam web is released to cause a contraction of the foam web. The adhesive retains the wadding product and foam together while permitting bulking in areas between the adhesive zones. The stresses still remaining in the product after contraction may be further relieved by wetting.

U.S. patent 3,842,832 to Wideman is directed to a disposable stretch product such as a bandage and a method for production of the product. The product is manufactured by passing a longitudinally oriented nonwoven material over a roller so as to apply an adhesive to one surface of the nonwoven material. At the same time a polyurethane web is heated and longitudinally stretched and adhered to the nonwoven material. Thereafter, a second nonwoven material is adhered to the other surface of the polyurethane web to form a laminate consisting of a stretched inner polyurethane core and outer unstretched nonwoven fabric layers adhered to the core by the adhesive. Next, the laminate is passed through a moistening device which results in a relaxing of the engagement between the nonwoven fabric outer layers and the adhesive connecting the outer layers to the stretched polyurethane core layer. This allows the stretched polyurethane layer to return to substantially its original length which results in the outer nonwoven layers being buckled or undulated to form wrinkles.

U.S. patent 4,104,170 to Nedza discloses a liquid filter having an improved extended polypropylene element. Fabrication of the polypropylene element is accomplished by forming a spunbonded underlayer of a continuous polypropylene fiber which adheres to itself as it is laid down in a random pattern. Thereafter, an overlayer of short polypropylene fibers is deposited onto the underlayer by, for example, meltblowing the overlayer onto an extended sheet of the underlayer.

A method for producing an elastic cloth structure which includes fibers of a synthetic, organic, relatively elastomeric polymer and fibers of a synthetic, organic, elongatable, but relatively nonelastic polymer is disclosed in U.S. patent 4,209,563 to Sisson. The method includes the steps of forwarding the relatively elastic fibers and elongatable but relatively non-elastic fibers for a well dispersed random lay-down on a porous forming surface of an unbonded web having random fiber crossings. Thereafter, at least some of the fiber crossings are bonded to form a coherent bonded cloth web which is stretched to elongate some of the fibers in at least one direction and then released so that retraction of the web by the relatively elastomeric fibers provides for looping and bunching of the elongatable relatively nonelastic fibers. Forwarding of the fibers to the porous forming surface is positively controlled, and this positive control is contrasted at column 7, lines 19-33 of the patent to the use of air streams to convey the fibers. It is also stated at column 9, line 44 et. seq. of the patent that bonding of the filaments to form the coherent cloth may utilize embossing patterns or smooth heated roll nips.

U. S. Patent 4,296,163 to Emi et al. discloses a fibrous composite having a coalcesed assembly of (A) a sheet-like mesh structure composed of fibers of a synthetic elastomeric polymer, the individual fibers of which are interconnected at random in irregular relationship to form a number of meshes of different sizes and shape with the mesh structure having a recovery ratio after 10% stretch of at least 70% in two arbitrarily selected, mutually perpendicular directions on the plane of the mesh structure, and (B) a mat-, web- or sheet-like fiber structure composed of short or long fibers, with the fiber structure having a recovery ratio after 10% stretch of less than 50% in at least one arbitrarily selected direction. It is stated that the elastic composite is suitable as various apparel based materials and industrial materials such as filter cloths, absorbents, and heat insulating materials. Methods for forming the composite are described at column 6, line 64 et seq. and these methods include spun bonding, see column 9, lines 15 - 41.

U.S. patent 4,323,534 to DesMarais discloses an extrusion process for a thermoplastic resin composition for fabric fibers with exceptional strength and good elasticity. At column 8 under the subtitle "Fiber-Forming" meltblowing of a compounded resin comprising 79.13% KRATON® G-1652, 19.78% stearic acid, 0.98% titanium dioxide and 0.1% Irganox® 1010 antioxidant is disclosed. It is stated that individual fibers were extruded from the meltblowing die.

U.S. patent 4,355,425 to Jones discloses a panty with a built-in elastic system to minimize gathering and to provide a comfortable, conforming fit and a method for assembling the panty. It is stated that a material made of meltblown KRATON® rubber is well suited for the panty fabric material. It is also stated that a process for making meltblown KRATON® fabrics is disclosed and shown schematically in figure 8 of the patent. The process which appears to utilize KRATON® G-1652 is discussed starting at column 4, line 67 of the patent.

U.S. patent 4,379,192 to Wahlquist discloses a method for forming an impervious absorbent barrier fabric embodying film and fibrous webs where one or more meltblowing dies meltblow discontinuous fibers of small diameter as a mat directly on a prebonded web of continuous filaments. At column 3, lines 35-40 of the patent it is stated that by forming the microfiber mat directly onto the prebonded continuous filament web, primary bonds are created between the microfibers and the continuous filaments which attach the microfiber mat to the continuous filament web.

U.S. patent 4,426,420 to Likhyani discloses hydraulically entangled spunlaced fabrics composed of at least two types of staple fibers and processes for their formation which include heat treating elastomeric fibers, which behave as ordinary staple fibers until they are heat treated, to impart improved stretch and resilience properties to the fabric. The method includes the steps of drawing a potentially elastomeric fiber and allowing it to relax between the drawing and wind-up steps.

U.S. patent 4,446,189 to Romanek discloses a nonwoven textile fabric laminate which includes at least one layer of nonwoven textile fabric which is secured by needle punching to an elastic layer so that the nonwoven layer of textile fabric will be permanently stretched when the elastic layer is drafted within its elastic limits. When the elastic layer is allowed to relax and return to substantially its condition prior to being drafted the nonwoven fabric layer is stated to exhibit increased bulk as a result of its concurrent relaxation. It is also stated that the nonwoven textile fabric laminate may be utilized to form wearing apparel which has enhanced freedom of movement.

The abstract of Japanese document number 47-43150 discloses a method for producing a nonwoven fabric having high tenacity with the method being carried out by (a) monoaxially stretching a sheet or film made of a mixture of incompatible polymers, (b) laminating this sheet or material with a layer of foamed polymer, (c) stretching the laminate at right angles to the direction of orientation of the substrate and then (d) stretching in the direction orientation of the substrate. Preferred polymers are stated to include polyamides, linear polyesters, and polyolefins. Preferably, the upper layer is a polypropylene foam.

A Shell Chemical Company brochure entitled "KRATON® Thermoplastic Rubber" generally discusses thermoplastic KRATON® materials. This brochure is code designated by "SC: 198-83 printed in U.S.A. 7/83 SM".

It is the object underlying the present invention to provide a novel process for producing a composite nonwoven elastic web comprising a nonwoven elastic web joined to a fibrous nonwoven gathered web, and a novel process for producing a gathered nonwoven web, whereby the materials obtained are elastic and have an excellent softness and breathability as well as excellent water repelling properties.

According to the present invention this object is attained with:
(1) a process for producing a composite nonwoven elastic web comprising a nonwoven elastic web joined to a fibrous nonwoven gathered web, comprising the step of:
   (a) providing a nonwoven elastic web,
      **characterized in that** it further comprises the steps of
   (b) stretching said nonwoven elastic web from at least about 125% of the relaxed length of the nonwoven elastic web to about 700% of the relaxed length of the nonwoven elastic web;
   (c) forming a fibrous nonwoven gatherable web directly upon a surface of the stretched nonwoven elastic web and joining the stretched fibrous nonwoven gatherable web to the stretched nonwoven elastic web so as to form a composite nonwoven elastic web; and
   (d) relaxing the composite nonwoven elastic web to gather the fibrous nonwoven gatherable web, and
(2) a process for producing a gathered nonwoven web having elastic characteristics, comprising the step of:
   a) providing an extendable and contractable forming surface,
      **characterized in that** it further comprises the steps of
   b) extending the forming surface from at least about 125% to about 700% of its unextended length;
   c) forming a fibrous nonwoven gatherable web directly upon the extended forming surface to separably join the fibrous nonwoven gatherable web to the extended forming surface;
   d) contracting the forming surface to gather the fibrous nonwoven gatherable web; and
   e) separating the gathered fibrous nonwoven gatherable web from the contracted forming surface.

Preferred embodiments of the present invention are set out in the dependent claims.

### DEFINITIONS

The terms "elastic" and "elastomeric" are used interchangeably herein to mean any material which, upon application of a biasing force, is stretchable to a stretched, biased length which is at least about 125%, that is about one and one quarter, of its relaxed, unbiased length, and which will recover at least about 40% of its elongation upon release of the stretching, elongating force. A hypothetical example which would satisfy this definition of an elastomeric material would be a 2.54 cm (one (1) inch) sample of a material which is elongatable to at least 3.18 cm (1.25 inches) and which, upon being elongated to 3.18 cm (1.25 inches) and released will recover to a length of not more than 2.92 cm 1.15 inches. Many elastic materials may be stretched by much more than 25% of their relaxed length and many of these will recover to substantially their original relaxed length upon release of the stretching, elongating force and this latter class of materials is generally preferred for purposes of the present invention.

As used herein the term "recover" refers to a contraction of a stretched material upon termination of a biasing force following stretching of the material by application of the biasing force. For example, if a material having a relaxed, unbiased length of 2.54 cm (one (1) inch) was elongated 50% by stretching to a length of 3.81 cm (one and one half (1.5) inches) the material would have a stretched length that is 150% of its relaxed length. If this exemplary stretched material contracted, that is recovered, to a length of 2.79 cm (one and one tenth (1.1) inches), after release of the biasing and stretching force, the material would have recovered 80% 1.02 cm (0.4 inch) of its elongation.

As used herein the terms "nonelastic" or "nonelastomeric" refer to and include any material which is not encompassed by the terms "elastic" or "elastomeric."

As used herein the term "meltblown microfibers" refers to small diameter fibers having an average diameter not greater than about 100 µm, preferably having a diameter of from about 0.5 µm to about 50 µm, more preferably having an average diameter of from about 4 µm to about 40 µm and which are made by extruding a molten thermoplastic material through a plurality of fine, usually circular, die capillaries as molten threads or filaments into a high velocity gas (e.g. air) stream which attenuates the filaments of molten thermoplastic material to reduce their diameter to the range stated above. Thereafter, the meltblown microfibers are carried by the high velocity gas stream and are deposited on a collecting surface to form a web of randomly disbursed meltblown microfibers. Such a process is disclosed, for example, in U.S. patent 3,849,241 to Butin and the disclosure of this patent is hereby incorporated by reference.

As used herein the term "spunbonded microfibers" refers to small diameter fibers having a diameter not greater than about 100 µm, preferably having a diameter of from about 10 µm to about 50 µm, more preferably having a diameter of from about 12 µm to about 30 microns and which are made by extruding a molten thermoplastic material as filaments through a plurality of fine, usually circular, capillaries of a spinnerette with the diameter of the extruded filaments then being rapidly reduced as by, for example, eductive drawing or other well known spunbonding mechanisms. The production of spunbonded nonwoven webs is illustrated in U.S. patent 4,340,563 to Appel and the disclosure of this patent is hereby incorporated by reference.

As used herein the term "nonwoven web" includes any web of material which has been formed without use of textile weaving processes which produce a structure of individual fibers which are interwoven in an identifiable repeating manner. Specific examples of nonwoven webs would include, without limitation, a meltblown nonwoven web, a spunbonded nonwoven web, an apertured film, a microporous web or a carded web of staple fibers. These nonwoven webs have an average basis weight of not more than about 300 g/m². Preferably, the nonwoven webs have an average basis weight of from about 5 g/m² to about 100 g/m². More preferably, the nonwoven webs have an average basis weight of from about 10 g/m² to about 75 g/
As used herein the term "consisting essentially of" does not exclude the presence of additional materials which do not significantly affect the elastomeric properties and characteristics of a given composition. Exemplary materials of this sort would include, pigments, anti-oxidants, stabilizers, surfactants, waxes, flow promoters, solid solvents, particulates and materials added to enhance processability of the composition.

As used herein the term "styrenic moiety" means a monomeric unit represented by the formula:

Unless specifically set forth and defined or otherwise limited, the terms "polymer" or "polymer resin" as used herein generally include, for example, homopolyers, copolymers, such as, for example, block, graft, random and alternating copolymers and terpolymers, and blends and modifications thereof. Furthermore, unless otherwise specifically limited, the terms "polymer" or "polymer resin" shall include all possible geometrical configurations of the material. These configurations include, for example, isotactic, syndiotactic and random symmetries.

An important feature of the process of the present invention is that the fibrous nonwoven gatherable web is formed directly onto a surface of the nonwoven elastic web while the nonwoven elastic web is maintained in a stretched, biased and elongated condition.

The nonwoven elastic web may be formed by, for example, a meltblowing process or any other process for forming a nonwoven elastic web. For example, the nonwoven elastic web could be an apertured web of an elastic film as opposed to a meltblown fibrous nonwoven elastic web. The formed nonwoven elastic web has a normal relaxed, nonstretched, nonbiased length. Thereafter, the nonwoven elastic web is elongated by being stretched.

In a subsequent step of the process the fibrous nonwoven gatherable web is formed, for example, by either a meltblowing or spunbonding process or any other process for forming a fibrous nonwoven gatherable web, directly upon the surface of the nonwoven elastic web while the nonwoven elastic web is maintained at its elongated, stretched and biased length.

Because the fibrous nonwoven gatherable web is formed directly onto the surface of the nonwoven elastic web while the nonwoven elastic web is being maintained at its stretched, biased length, the nonwoven elastic web is, at this stage in the process, elongated, stretched and biased and the fibrous nonwoven gatherable web is in an ungathered but gatherable condition.

In one embodiment of the present invention, joining of the fibrous nonwoven gatherable web to the nonwoven elastic web is achieved by heat-bonding to fuse the two webs to each other. The heat-bonding may be carried out within the temperature range of from about 50 °C below the melt temperature of at least one of the materials utilized to form at least one of the two webs to about the melt temperature of at least one of the materials utilized to form at least one of the two webs. At high through-put rates the heat-bonding can be carried out above the melt temperature of one or more of the materials utilized to form the webs. The heat-bonding may also be carried out under appropriate conventional pressurized conditions. If desired, conventional sonic bonding techniques may be substituted for the heat-bonding steps.

In another embodiment of the present invention joining of the fibrous nonwoven gatherable web to the stretched nonwoven elastic web is achieved solely by the entanglement of the individual fibers of the fibrous nonwoven gatherable web with the nonwoven elastic web during formation of the fibrous gatherable web on the surface of the elastic web. If the nonwoven elastic web is a fibrous nonwoven elastic web formed by, for example, meltblowing, entanglement of the individual fibers of the fibrous nonwoven gatherable web with the fibrous nonwoven elastic web is achieved by entanglement of the individual fibers of the fibrous gatherable web with the individual fibers of the fibrous elastic web. If the nonwoven elastic web is an apertured film, joining of the fibrous nonwoven web with the film is achieved by entanglement of the individual fibers of the fibrous gatherable web within the apertures of the film.

In yet another embodiment, discussed below, the joining of the two webs to each other is achieved by also forming the nonwoven elastic web out of a tacky elastic material.

In any of the embodiments of the present process joining of the two webs to each other may be further enhanced by applying pressure to the two webs after the gatherable web has been formed on the surface of the elastic web. Also, in any embodiment, joining of the two webs may be further improved by applying an adhesive material to the upper surface of the nonwoven elastic web prior to formation of the fibrous nonwoven gatherable web thereon.

After joining of the two webs to each other has been achieved to form a composite elastic web, the biasing force is removed from the composite nonwoven elastic web and the composite elastic web is allowed to relax to its normal relaxed, unbiased length. Because the fibrous nonwoven gatherable web is joined to the nonwoven elastic web while the nonwoven elastic web is stretched, relaxation of the composite nonwoven elastic web results in the gatherable web being carried with the contracting nonwoven elastic web and thus being gathered.

After gathering of the fibrous nonwoven gatherable web has occurred by reducing the biasing force on the composite nonwoven elastic web, the composite nonwoven elastic web may be rolled up in rolls for storage and shipment. The composite elastic web may thereafter be utilized to form a wide range of products, such as, for example, an outer cover for a diaper.

Alternatively the gathered nonwoven web may be separated from the nonwoven elastic web subsequent to its being gathered by the retractive forces of the nonwoven elastic web. In this embodiment the gathered nonwoven web can be utilized alone or in conjunction with a variety of other webs or film materials to form numerous different products. Interestingly, the separated gathered nonwoven web retains a substantial degree of its gathered configuration and also exhibits elastic properties. The gathered nonwoven web may be formed, as discussed above, in a gatherable condition directly onto the surface of the elastic nonwoven web with the elastic nonwoven web being in an extended state.

Upon its formation on the surface of the nonwoven elastic web, the fibrous nonwoven gatherable web is separably joined to the nonwoven elastic web while the nonwoven elastic web is maintained at its extended stretched, biased length. This results in the formation of a composite nonwoven elastic web which includes the nonwoven elastic web and the fibrous nonwoven gatherable web with the fibrous nonwoven gatherable web being separably joined to the nonwoven elastic web. Because the fibrous nonwoven gatherable web is formed directly onto the surface of the nonwoven elastic web while the nonwoven elastic web is being maintained at its extended stretched, biased length, the nonwoven elastic web is, at this stage in the process, extended, stretched and biased and the fibrous nonwoven gatherable web is in an ungathered but gatherable condition.

The separable joining of the fibrous nonwoven gatherable web to the extended, stretched nonwoven elastic web is achieved by the entanglement of the individual fibers of the fibrous nonwoven gatherable web with the nonwoven elastic web during formation of the fibrous nonwoven gatherable web on the surface of the nonwoven elastic web. If the nonwoven elastic web is a fibrous nonwoven elastic web formed by, for example, meltblowing, the separable joining of the fibrous nonwoven gatherable web to the fibrous nonwoven elastic web is achieved by entanglement of the individual fibers of the fibrous gatherable web with the individual fibers of the fibrous nonwoven elastic web. If the nonwoven elastic web is an apertured film, the separable joining of the fibrous nonwoven web with the nonwoven elastic web is achieved by entanglement of the individual fibers of the fibrous gatherable web within the apertures of the apertured film.

After the separable joining of the two webs to each other has been achieved to form the composite elastic web, the biasing force is removed from the composite nonwoven elastic web and the composite elastic web is allowed to contract, due to contraction of the stretched nonwoven elastic web, to its normal contracted, unbiased length. Because the fibrous nonwoven gatherable web is separably joined to the nonwoven elastic web while the nonwoven elastic web is extended and stretched, contraction of the composite nonwoven elastic web results in the gatherable web being carried with the contracting nonwoven elastic web and thus being gathered on the surface of the nonwoven elastic web.

After gathering of the fibrous nonwoven gatherable web has occurred by reducing the biasing force on the composite nonwoven elastic web the gathered fibrous nonwoven web is separated from the nonwoven elastic web and the gathered web may, for example, be rolled up for storage. After separation of the fibrous nonwoven gathered web from the nonwoven elastic web, the nonwoven elastic web may be reused as a forming surface.

Upon its separation from the nonwoven elastic web, the fibrous nonwoven gathered web retains a gathered configuration and, upon application of a stretching and biasing force in the direction in which the fibrous nonwoven gatherable web was gathered, the gathered web extends to the extent that the gathers allow. Importantly, upon release of the stretching and biasing force the extended, fibrous nonwoven gathered web contracts substantially to the gathered configuration and length which it possessed after its separation from the nonwoven elastic web. That is, the fibrous nonwoven gathered web exhibits elastic characteristics and properties. The fact that the gathered web, upon its separation from the nonwoven elastic web, retains a gathered configuration is surprising. However, it is even more surprising that the separated fibrous nonwoven gathered web, upon being stretched to an extended length, exhibits elastic properties such as recovering at least about 40% of its elongation. That is, the separated fibrous nonwoven web exhibits elastic or elastomeric properties as defined herein. In fact, it has been found that the fibrous nonwoven gathered web exhibits these elastic properties even when the fibrous nonwoven gathered web was formed from a nonelastic material such as polypropylene.

Preferably, the fibrous nonwoven gatherable web includes at least one meltblown fibrous nonwoven web. Alternative methods which may be utilized in forming the fibrous nonwoven gatherable web include spunbonding or any other process for forming a fibrous nonwoven gatherable web. The gathered fibrous nonwoven web may be formed entirely from one nonelastic material or from a blend of one or more nonelastic materials. However, the gathered fibrous nonwoven may be formed from blends of one or more nonelastic materials with one or more elastic materials or from one or more elastic materials. Nonelastic materials for forming the fibrous nonwoven gatherable web include nonelastic polyester materials, nonelastic polyolefin materials or blends of one or more nonelastic polyester materials with one or more nonelastic polyolefin materials. An exemplary nonelastic polyester material is polyethylene terephthalate. An exemplary nonelastic polyolefin is a nonelastic polypropylene which may be obtained under the trade designation PF 301.

Alternatively, the necessity for the elastic nonwoven web can be eliminated by forming the gathered nonwoven web in a gatherable condition directly onto an extensible and contractable surface, such as, for example, an extendable and retractable mesh screen, as in the second process of the present invention.

In one particular embodiment of the process of the present invention a tacky fibrous nonwoven elastic web is formed by, for example, meltblowing microfibers of a tacky elastic material such as, for example, an A-B-A' block copolymer or blends of such A-B-A' block copolymers with poly (alpha-methylstyrene) where A and A' are each thermoplastic polystyrene or polystyrene homologue end blocks and B is an elastic polyisoprene midblock. In some embodiments A may be the same thermoplastic polystyrene or polystyrene homologue endblock as A'. The tacky fibrous nonwoven elastic web is then elongated by being stretched to an elongated, stretched length and a fibrous nonwoven gatherable web is formed, for example, by meltblowing or spunbonding the fibrous nonwoven gatherable web, directly upon a surface of the tacky fibrous nonwoven elastic web while maintaining the fibrous nonwoven elastic web at its stretched length. As a result of the fact that the fibrous nonwoven elastic web is tacky, the fibrous nonwoven gatherable web is simultaneously formed upon and adhesively joined to the surface of the tacky fibrous nonwoven elastic web. This embodiment results in the formation of a composite nonwoven elastic web having an ungathered fibrous gatherable web adhesively joined to the tacky fibrous nonwoven elastic web with the joining of the two webs to each other being achieved by the adhesive joining which occurs during formation of the fibrous nonwoven gatherable web on the surface of the fibrous nonwoven elastic web. The adhesive joining of the two webs to each other may be increased upon application pressure to the composite nonwoven elastic web by passing the composite nonwoven elastic web through the nip between rollers, which may be unheated, after the composite web has been formed but before the fibrous tacky nonwoven elastic web is allowed to relax. The adhesive joining may be further enhanced by application of an adhesive material to the surface of the tacky fibrous nonwoven elastic web prior to formation of the gatherable web thereon.

The composite nonwoven elastic web is then allowed to relax to its normal relaxed, unbiased length. Because the fibrous nonwoven gatherable web was joined to the tacky fibrous nonwoven elastic web while the tacky fibrous nonwoven elastic web was in a stretched condition, relaxation of the composite nonwoven elastic web and thus the tacky fibrous nonwoven elastic web results in the gatherable web being carried with the contracting fibrous nonwoven elastic web and thus being gathered.

After gathering of the fibrous nonwoven gatherable web has occurred the composite nonwoven elastic web may be rolled up in rolls for storage and shipment. In order to avoid adhesion of the exposed side of the tacky fibrous nonwoven elastic web upon rolling-up of the composite nonwoven elastic web it is preferred for a second fibrous nonwoven gatherable web to be applied to the exposed surface of the fibrous nonwoven elastic web prior to the gathering step. Alternatively, butcher paper may be applied, either before or after gathering of the gatherable web, to the exposed tacky surface of the tacky fibrous nonwoven elastic web and later removed prior to utilization of the composite nonwoven elastic web. The composite elastic web may thereafter be utilized to form a wide variety of products.

Exemplary elastomeric materials for use in formation of the fibrous nonwoven elastic web include polyester elastomeric materials, polyurethane elastomeric materials, and polyamide elastomeric materials. Other elastomeric materials for use in formation of the fibrous nonwoven elastic web include (a) A-B-A' block copolymers, where A and A' are each a thermoplastic polymer endblock which includes a styrenic moiety and where A may be the same thermoplastic polymer endblock as A', such as a poly (vinyl arene), and where B is an elastomeric polymer midblock such as a conjugated diene or a lower alkene or (b) blends of one or more polyolefins or poly (alpha-methyl styrene) with A-B-A' block copolymers, where A and A' are each a thermoplastic polymer endblock which includes a styrenic moiety, where A may be the same thermoplastic polymer endblock as A', such as a poly (vinyl arene) and where B is an elastomeric polymer midblock such as a conjugated diene or a lower alkene. The A and A' endblocks may be selected from the group including polystyrene and polystyrene homologs and the B midblock may be selected from the group including polyisoprene, polybutadiene or poly (ethylene-butylene). If A and A' are selected from the group including polystyrene or polystyrene homologs and B is poly (ethylene-butylene), materials which may be blended with these block copolymers are polymers, including copolymers of ethylene, propylene, butene, other lower alkenes or one or more of these materials. If A and A' are selected from the group including polystyrene or polystyrene homologs and B is a polyisoprene midblock, a material for blending with this type of block copolymer is poly (alpha-methylstyrene).

Preferably, the gatherable web includes at least one fibrous nonwoven web that includes nonelastic fibers which may be formed by meltblowing, spunbonding, or any other process for forming a fibrous nonwoven gatherable web. Preferred materials for forming the gatherable web include polyester materials, polyolefin materials or blends of one or more polyester materials with one or more polyolefin materials. An exemplary polyester material is polyethylene terephthalate. An exemplary polyolefin material is polypropylene.

### BRIEF DESCRIPTION OF THE DRAWINGS

Figure 1 is a schematic view illustrating one mode for carrying out the method of one of the embodiments of the present invention.

Figure 2 is a schematic view illustrating a mode for carrying out the method of another of the embodiments of the present invention.

Figure 3 is a schematic view illustrating one mode for carrying out the method of an embodiment of the present invention where the gathered web is separated from the elastic web.

Figure 4 is a schematic view illustrating another mode for carrying out the method of another embodiment of the present invention where the gathered web is separated from the elastic web.

Figure 5 is a top plan view of an unbiased and retracted extendable and retractable forming screen which may be utilized as a forming screen in the process illustrated in Figure 4.

Figure 6 is a top plan view of the extendable and retractable forming screen of Figure 5 in the biased, extended configuration.

Figure 7 is a schematic view of yet another mode for carrying out the method of yet another embodiment of the present invention where the two gathered webs are separated from the elastic web.

Turning now to the figures wherein like reference numerals represent like structure and, in particular, to figure 1, it can be seen that meltblown microfibers 10 which are formed by a conventional meltblowing die 12 are collected on a porous collecting screen 14 which is moving, as indicated by the arrows 16 in figure 1, about the rollers 18 and 20. The material which is utilized to form the meltblown microfibers 10 is, for reasons which will hereinafter become clear, an elastomeric material. The porous collecting screen 14 is driven by the rotating rollers 18 and 20 which, in turn, are driven by a conventional drive arrangement (not shown). Also not shown for purposes of clarity is a conventional vacuum box located between the rollers 18 and 20 and beneath the lower surface of the upper portion of the screen 14. The vacuum box assists in the retention of the microfibers 10 on the upper surface of the screen 14. As the meltblown microfibers 10 are deposited upon the moving collecting screen 14 they entangle and cohere to form a cohesive fibrous nonwoven elastic web 22. The entangled cohesive fibrous nonwoven elastic web 22 is carried by the porous collecting screen 14 to the nip or gap 24 between the rotating roller 20 and a rotating nip roller 26. The nip or gap 24 between the two rollers 20 and 26 is adjusted so that the rollers 20 and 26 firmly engage the fibrous nonwoven elastic web 22 without adversely affecting the web 22. The rate of rotation of the rollers 20 and 26 is adjusted so that the peripheral surface speed of the rollers 20 and 26 is substantially the same as the speed of the moving porous collecting screen 14. If, upon lay-down on the surface of the porous screen 14, the meltblown microfibers 10 are insufficiently cohered to each other to form a cohesive web 22 capable of performing the hereinafter discussed stretching and relaxing steps without being adversely affected (e.g. the web separates, loses it integrity, upon application of a stretching force), the cohesion of the microfibers 10 to each other may be improved by, for example, heat-bonding the microfibers 10 to each other by maintaining the roller 26 at an appropriate elevated temperature which will vary depending upon the degree of cohesion desired and the cohesive characteristics of the material utilized to form the microfibers 10. Typical heat-bonding temperatures range from about 50 °C below the melting temperature of at least one of the materials utilized to form the web 22 to about the melting temperature of at least one of the materials utilized to form the web 22. However, at high throughput rates temperatures exceeding the melting temperature of the material may be employed. After passing through the nip 24 the fibrous nonwoven elastic web 22 is forwarded by the action of the rollers 20 and 26 into and passes through a second nip or gap 28 which is formed between a rotating roller 30 and a second rotating nip roller 32. Rotation of the rollers 30 and 32 is adjusted so that the peripheral surface speed of the rollers 30 and 32 is greater than the peripheral surface speed of the rollers 20 and 26. The nip 28 between the two rollers 30 and 32 is adjusted so that the rollers 30 and 32 firmly engage the fibrous nonwoven elastic web 22 without adversely affecting the web 22. As a result of the increase in the peripheral surface speed of the rollers 30 and 32 with respect to the peripheral surface speed of the rollers 20 and 26 a longitudinal or machine direction (MD) biasing force is placed on the fibrous nonwoven elastic web 22 and the web 22 is stretched to an extended, stretched, biased length in the longitudinal or machine direction (MD). The degree of stretching of the fibrous nonwoven elastic web 22 which occurs in the area 34 between the rollers 20 and 26 and the rollers 30 and 32 may be varied, for example, by varying the peripheral surface speed of the rollers 30 and 32 with respect to the peripheral surface speed of the rollers 20 and 26. For example, if the peripheral surface speed of the rollers 30 and 32 is twice that of the rollers 20 and 26, the fibrous nonwoven elastic web 22 will be stretched to a stretched length of substantially about twice, that is, about 200%, of its original relaxed unstretched, unbiased length. The fibrous nonwoven web 22 is stretched to a stretched length of at least about 125% of its original, relaxed, unbiased length, preferably from at least about 150% of the relaxed, unbiased length of the fibrous nonwoven web 22, to about 700% or more of the relaxed, unbiased length of the fibrous nonwoven web 22.

After the fibrous nonwoven elastic web 22 has been stretched, by the combined actions of rollers 20 and 26 and 30 and 32, the web 22 is passed onto a second porous collecting screen 36 which is moving as is indicated by the arrows 38 in figure 1. The second porous collecting screen 36 moves about and is driven by the rotating roller 30 in conjunction with a rotating roller 40. The rotating rollers 30 and 40 are, in turn, driven by a conventional driving arrangement (not shown) which may be the same arrangement that is driving the rotating rollers 18 and 20. Also not shown for purposes of clarity is a conventional vacuum box located between the rollers 30 and 40 and beneath the lower surface of the upper portion of the screen 36. The vacuum box assists in the retention of the web 22 on the upper surface of the screen 36. The stretched fibrous nonwoven elastic web 22 is carried by the second porous collecting screen 36 to a nip or gap 42 which is formed between the rotating roller 40 and a third rotating nip roller 44. Rotation of the rotating roller 40 and the nip roller 44 is adjusted so that the peripheral surface speed of the two rollers 40 and 44 is substantially the same as the peripheral surface speed of the rollers 30 and 32. Because the peripheral surface speed of the rollers 40 and 44 is maintained at substantially the same peripheral surface speed as that of the rollers 30 and 32 and because the nip 42 is adjusted so that the rollers 40 and 44 firmly retain the fibrous nonwoven elastic web 22, without adversely affecting the web 22, the stretched condition of the fibrous nonwoven elastic web 22 is maintained while the fibrous nonwoven elastic web 22 is being carried by the second porous collecting screen 36.

While the stretched fibrous nonwoven elastic web 22 is being carried by the second porous collecting screen 36 meltblown microfibers 46, formed by a conventional meltblowing die 48, are meltblown directly onto the upper surface of the stretched nonwoven elastic web 22 to form a cohesive fibrous nonwoven gatherable web 50 which is located on the upper surface of the stretched fibrous nonwoven elastic web 22. Care should be taken to adjust the distance between the die tip of the meltblowing die 48 and the elastic web 22 and the speed at which the elastic web 22 passes under the die tip of the meltblowing die 48, as it has been found that the hot air exiting the die tip will melt the elastic web 22 if these adjustments, which will vary with the material or blend of materials from which the elastic web 22 is formed, are not properly made. As the meltblown microfibers 46 are collected on the upper surface of the fibrous nonwoven elastic web 22, they entangle and cohere with each other to form the cohesive fibrous nonwoven gatherable web 50. Depending upon the distance between the die tip of the meltblowing die 48 and the upper surface of the stretched fibrous nonwoven elastic web 22 the meltblown microfibers 46 may also mechanically entangle with the fibers of the elastic web 22. Generally speaking, as the distance between the die tip of the meltblowing die 48 and the upper surface of the stretched fibrous nonwoven elastic web 22 is increased the mechanical entanglement of the fibers of the web 50 with the fibers of the web 22 decreases. To assure mechanical entanglement of the fibers of the web 50 with the fibers of the web 22 the distance between the die tip of the meltblowing die 48 and the upper surface of the web 22 should be no greater than about 63.5 cm (25 inches). Preferably, the distance between the die tip of the meltblowing die 48 and the upper surface of the web 22 should range from about 15.24 cm (6 inches) to about 40.64 cm (16 inches). Depending on the materials utilized to form the webs 22 and 50 and the distance between the die tip of the meltblowing die 48 and the upper surface of the web 22 some adhesion of the fibers of the gatherable web 50 to the fibers of the elastic web 22 may also occur. The materials which are appropriate for utilization in forming the fibrous nonwoven elastic web 22 are preferably selected after selection of the material or materials which will be utilized in formation of the fibrous nonwoven gatherable web 50 has occurred. In particular, the material selected to form the fibrous nonwoven gatherable web 50 must be a material which forms a web 50 that is gatherable by the contracting force of the fibrous nonwoven elastic web 22. Because the contracting force of the web 22 will vary with the material selected for formation of the web 22, the material selected for formation of the web 22 will have to be selected so that the contracting force of the web 22 is capable of gathering the web 50. Exemplary, materials for utilization in forming the webs 22 and 50 are disclosed hereinafter.

Depending upon the characteristics which are desired for the final product, the materials which are utilized to form the fibers which compose the two webs 22 and 50 and the process steps/conditions utilized, the two cohesive webs 22 and 50 may be joined to each other in a variety of ways. For example, if a relatively weak joining of the two webs 22 and 50 to each other is desired, the two webs 22 and 50 can be joined to each other solely by the entanglement of the individual meltblown fibers of the fibrous nonwoven gatherable web 50 with the individual meltblown fibers of the fibrous nonwoven elastic web 22 which occurs during formation of the web 50 on the stretched surface of the web 22. In this embodiment, the two webs 22 and 50 are separable from each other upon application of a relatively small amount of force such as, for example, a light picking or rubbing force applied by an individual's fingers. In the event that a stronger joining of the two cohesive webs 22 and 50 to each other is desired, joining of the fibrous nonwoven gatherable web 50 to the fibrous nonwoven elastic web 22 can be achieved, while continuing to maintain the fibrous nonwoven elastic web 22 at its stretched length, by heat-bonding the two webs 22 and 50 to each other. The heat-bonding can be achieved by, for example, passing the two webs 22 and 50 between the rollers 40 and 44 with the rollers 40 and 44 being arranged to apply appropriate heat-bonding temperatures and pressures to the two webs 22 and 50. For example, joining of the fibrous nonwoven gatherable web 50 to the fibrous nonwoven elastic web 22 may be achieved by heat-bonding of the two webs 22 and 50 to each other with the rollers 40 and 44 being maintained within the temperature range of from about 50 °C below the melting point of at least one of the materials used to form the web 22 and 50 to about the melt temperature of at least one of the materials utilized to form the webs 22 and 50. However, at high through-put rates the heat-bonding can be carried out above the melt temperature of one or more of the materials utilized to form the two webs 22 and 50 since the webs 22 and 50 will be exposed to the high temperature for a short time. Pressurized heat-bonding of the two webs 22 and 50 to each other may be carried out at conventional, appropriate bonding pressures by adjusting the nip 42. Other conventional alternatives to heat-bonding the two webs 22 and 50 to each other may be substituted for the heat-bonding steps. For example, a conventional sonic bonding arrangement (not shown) could be substituted for the heat-bonding arrangement 40 and 44. It should be noted that the joining of the two webs 22 and 50 to each other is usually improved somewhat just by passage of the webs 22 and 50 through the nip 42 since such passage results in application of pressure to the two webs 22 and 50 and thus increased entanglement of the individual fibers of the two webs 22 and 50.

After the fibrous nonwoven elastic web 22 has been joined (separably or nonseparably, depending upon the final product which is desired) to the fibrous nonwoven gatherable web 50 to form a composite nonwoven elastic web 52 the biasing force on the fibrous nonwoven elastic web 22 is relaxed by, for example, passing the composite nonwoven elastic web 52, which includes both the fibrous nonwoven elastic web 22 and the fibrous nonwoven gatherable web 50, through the nip or gap 54 formed by a pair of rotating nip rollers 56 and 58. The nip 54 is adjusted so that the rollers 56 and 58 firmly engage the composite web 52 without adversely affecting the composite web 52. The rotation of the pair of nip rollers 56 and 58 is adjusted so that the peripheral surface speed of the nip rollers 56 and 58 allows the composite nonwoven elastic web 52 to relax and, as a result of its elastic properties, to contract to its relaxed, unbiased length. The relaxing and contracting of the composite nonwoven elastic web 52 to its relaxed, unbiased length results in the fibrous nonwoven gatherable web 50, which is joined to the fibrous nonwoven elastic web 22, being carried along with, that is contracted, and thus gathered upon the upper surface of the contracting fibrous nonwoven elastic web 22.

After relaxing and contracting of the composite nonwoven elastic web 52, the composite web 52 may be rolled up on a supply roller 60 for storage and shipment. The composite nonwoven elastic web 52 may thereafter be utilized in the manufacture of wide variety of items such as, for example, an outer cover material for a diaper or other garment.

Alternatively, if the gathered nonwoven web 50 is to be separated from the elastic nonwoven web 22, separation of the two webs 22 and 50 from each other is effected in this embodiment by passing the fibrous nonwoven gathered web 50 through the nip 62 between two rotating nip rollers 64 and 66 and passing the nonwoven elastic web 22 through the nip 68 between two rotating nip rollers 70 and 72. The nips 62 and 68 are adjusted so that the rollers 64 and 66 engage the web 50 without adversely affecting the web 50 and the rollers 70 and 72 engage the web 22 without adversely affecting the web 22. After separation of the two webs 22 and 50, the two webs 22 and 50 are wound up on storage rolls 74 and 76, respectively. Care should be taken in winding up the fibrous nonwoven gathered web 50 so that the web 50 is not stored under high tension or biasing in an ungathered condition because, if the web 50 is stored in a rolled-up tensioned, ungathered condition it is believed that the web 50 will lose its ability to retain its gathers. Loss of the gathers in the web 50 will result in a loss of the elastic characteristics of the web 50. Accordingly, in order to retain the gathered condition of the web 50 while the web 50 is stored the rotation of the storage roll 76 should be adjusted so that the peripheral surface speed of the roll 76 is generally equal to or just slightly greater than the peripheral surface speed of the rollers 64 and 66.

Upon its separation from the nonwoven elastic web 22 the gathered fibrous nonwoven web 50 exhibits a creped or gathered appearance. Accordingly, upon application of an extending force in the machine direction (i.e. is a direction substantially perpendicular to the lines of gathering) the web 50 is extended to the extent that the gathers allow, e.g. until the web 50 has assumed a generally planar configuration as opposed to a gathered configuration and, surprisingly, upon release of the extending force on the gathers, the gathered web 50 exhibits elastic characteristics as defined herein. The gathered web 50 exhibits elastic characteristics even when the web 50 was formed from a nonelastic material such as a polypropylene obtained from the Himont Corporation under the trade designation PF 301.

The fibrous nonwoven elastic web 22 portion of the composite nonwoven elastic web 52 may be formed from any elastomeric material which may be formed into a fibrous nonwoven elastic web 22. Exemplary elastomeric materials for use in formation of the fibrous nonwoven elastic web 22 include polyester elastomeric materials such as, for example, polyester elastomeric materials available under the trade designation Hytrel® from E. I. DuPont DeNemours & Co., polyurethane elastomeric materials such as, for example, polyurethane elastomeric materials available under the trade designation Estane® from B. F. Goodrich & Co. and polyamide elastomeric materials such as, for example, polyamide elastomeric materials available under the trade designation Pebax® from the Rilsan Company. Other elastomeric materials for use in forming the fibrous nonwoven elastic web 22 include (a) elastomeric A-B-A' block copolymers, where A and A' are each a thermoplastic polymer endblock which includes a styrenic moiety and where A may be the same thermoplastic polymer endblock as A', for example, a poly (vinyl arene), and where B is an elastomeric polymer midblock such as conjugated diene or a lower alkene and (b) blends of one or more polyolefins or poly (alpha-methylstyrene) with elastomeric A-B-A' block copolymer materials, where A and A' are each polymer thermoplastic endblocks containing a styrenic moiety and where A may be the same thermoplastic polymer endblock as A', such as a poly (vinyl arene) and where B is an elastomeric polymer midblock, such as a conjugated diene or a lower alkene. The A and A' materials may be selected from the group of materials including polystyrene or polystyrene homologs and the B material may be selected from the group of materials including polyisoprene, polybutadiene and poly (ethylene-butylene). Materials of this general type are disclosed in U.S. patents 4,323,534 to Des Marais and 4,355,425 to Jones and in the aforementioned Shell brochure. Commercially available elastomeric A-B-A' block copolymers having a saturated or essentially saturated poly (ethylene-butylene) midblock "B" represented by the formula:
where x, y and n are positive integers, and polystyrene endblocks A and A' represented by the formula:
where n is a positive integer which may be the same or different for A and A', are sometimes referred to as S-EB-S block copolymers and are available under the trade designation KRATON® G, for example, KRATON® G 1650, KRATON® G 1652 and KRATON® GX 1657, from the Shell Chemical Company. Other elastomeric resins which may be utilized are A-B-A' block copolymers where A and A' are polystyrene endblocks, as defined above, and "B" is a polybutadiene midblock represented by the following formula:
where n is a positive integer. This material is sometimes referred to as a S-B-S block copolymer and is available under the trade designation KRATON® D, for example, KRATON® D 1101, KRATON® D 1102 and KRATON® D 1116, from the Shell Chemical Company. Another S-B-S block copolymer material may be obtained under the trade designation Solprene 418 from the Phillips Petroleum Company. Yet other elastomeric resins which may be utilized are A-B-A' block copolymers where A and A' are polystyrene endblocks, as defined above, and B is a polyisoprene midblock where the midblock is represented by the formula:
where n is a positive integer. These block copolymers are sometimes referred to as S-I-S block copolymers and are available under the trade designation KRATON® D, for example, KRATON® D 1107, KRATON® D 1111, KRATON® D 1112 and KRATON® D 1117, from the Shell Chemical Company.

A summary of the typical properties of the above-identified KRATON® D and KRATON® G resins at 23°C (74° Fahrenheit) is presented below in Tables I and II.

**TABLE I**

| KRATON® D | | | | | | | |
|---|---|---|---|---|---|---|---|
| PROPERTY | D-1101 | D-1102 | D-1107 | D-1111 | D-1112 | D-1116 | D-1117 |
| Tensile Strength, kN/m² (psi)¹ | 31.7 (4,600)² | 31.7 (4,600)² | 21.4 (3,100)² | 20.0 (2,900)² | 10.3 (1,500)² | 31.7 (4,600)⁵ | 8.3 (1,200)² |
| 300% Modulus kN/m² (psi)¹ | 2.8 (400) | 2.8 (400) | 0.7 (100) | 1.4 (200) | 0.5 (70) | 2.4 (350) | 0.4 (60) |
| Elongation, %¹ | 880 | 880 | 1,300 | 1,200 | 1,400 | 900 | 1,300 |
| Set at Break, % | 10 | 10 | 10 | 10 | 20 | 10 | 15 |
| Hardness, Shore A | 71 | 71 | 37 | 52 | 34 | 65 | 32 |
| Specific Gravity | 0.94 | 0.94 | 0.92 | 0.93 | 0.92 | 0.94 | 0.92 |
| Brookfield Viscosity, (Toluene Solution) 10⁻³ Pa s (cp) at 25°C (77°F) | 4,000³ | 1,200³ | 1,600³ | 1,300³ | 900³ | 9,000³ | 500³ |
| Melt Viscosity Melt Index, Condition G, g/10 min | 1 | 6 | 9 | - | - | - | - |
| Plasticizer Oil Content, %w | 0 | 0 | 0 | 0 | 0 | 0 | 0 |
| Styrene/Rubber⁶ Ratio | 31/69 | 28/72 | 14/86 | 21/79 | 14/86 | 21/79 | 17/83 |
| Physical Form | Porous Pellet | Porous Pellet | Pellet | Porous Pellet | Pellet | Porous Pellet | Pellet |

| | | | | | | | |
|---|---|---|---|---|---|---|---|
| ¹ ASTM method D412-tensile test jaw separation speed 25.4 cm (10 in)/min. | | | | | | | |
| ² Typical properties determined on film cast from a toluene solution. | | | | | | | |
| ³ Neat polymer concentration, 25%w. | | | | | | | |
| ⁵ Property determined by extrapolation to zero oil content of results measured on oil extended films cast from toluene solution. | | | | | | | |
| ⁶ The ratio of the sum of the molecular weights of the endblocks (A + A') to the molecular weight of the B midblock. For example, with respect to KRATON® G - 1650 the molecular weight of the endblocks (A + A') is 28 % of the molecular weight of the A-B-A' block copolymer. | | | | | | | |

**TABLE II**

| KRATON® G | | | |
|---|---|---|---|
| PROPERTY | G-1650 | G-1652 | GX-1657 |
| Tensile Strength, kN/m² (psi)¹ | 34.5 (5,000)² | 31.0 (4,500)² | 23.4 (3,400)² |
| 300% Modulus, kN/m² (psi)¹ | 5.5 (800) | 4.8 (700) | 2.4 (350) |
| Elongation, %¹ | 500 | 500 | 750 |
| Set at Break, % | - | - | - |
| Hardness, Shore A | 75 | 75 | 65 |
| Specific Gravity | 0.91 | 0.91 | 0.90 |
| Brookfield Viscosity, (Toluene Solution) 10⁻³ Pa s (cp) at 25°C (77°F) | 1,500⁴ | 550⁴ | 1,200⁴ |
| Melt Viscosity, Melt Index, Condition G, g/10 min | - | - | - |
| Plasticizer Oil Content, %w | 0 | 0 | 0 |
| Sytrene/Rubber⁶ Ratio | 28/72 | 29/71 | 14/86 |
| Physical Form | Crumb | Crumb | Pellet |

| | | | |
|---|---|---|---|
| ¹ ASTM method D412-tensile test jaw separation speed 25.4 cm (10 in)/min. | | | |
| ² Typical properties determined on film cast from a toluene solution. | | | |
| ⁴ Neat polymer concentration, 20%w. | | | |
| ⁶ The ratio of the sum of the molecular weights of the endblocks (A + A') to the molecular weight of the B midblock. For example, with respect to KRATON® G - 1650 the molecular weight of the endblocks (A + A') is 28 % of the molecular weight of the A-B-A' block copolymer. | | | |

Meltblowing of the S-EB-S KRATON® G block copolymers in pure, i.e. neat, form has proven to be difficult except at elevated temperatures and low through-puts such as from at least about 287.8°C (550 degrees Fahrenheit) to about 329.4°C (625 degrees Fahrenheit) or more and below at least about 0.14 g per die capillary per min. In order to avoid these elevated temperature and low through-put conditions, blending of certain materials with several of the different types of KRATON® G materials has proven to provide a satisfactory meltblowable material. For example, blends of certain polyolefin materials with the S-EB-S block copolymer has resulted in a meltblowable material. In particular, if a polyolefin is to be blended with the KRATON® G S-EB-S block copolymers, the polyolefin is preferably a polymer, including copolymers, of ethylene, propylene, butene, other lower alkenes or blends of one or more of these materials. A particularly preferred polyolefin for blending with the KRATON® G S-EB-S block copolymers is polyethylene and a preferred polyethylene may be obtained from U.S.I. Chemicals Company under the trade designation Petrothene® Na601. (Also referred to herein as PE Na601 or Na601.)

Information obtained from U.S.I. Chemical Company states that the Na601 is a low molecular weight, low density polyethylene for application in the areas of hot melt adhesives and coatings. U.S.I. has also stated that the Na601 has the following nominal values: (1) a Brookfield Viscosity, mPa·s (cP) at 150 °C of 8500 and at 190 °C of 3300 when measured in accordance with ASTM D 3236; (2) a density of 0.903 g/cm³ when measured in accordance with ASTM D 1505; (3) an equivalent Melt index of 2000 g /10 min when measured in accordance with ASTM D 1238; (4) a ring and ball softening point or 102 °C when measured in accordance with ASTM E 28; (5) a tensile of 5.7 kN/m² (850 pounds per square inch) when measured in accordance with ASTM D 638; (6) an elongation of 90 % when measured in accordance with ASTM D 638; (7) a modulus of Rigidity, T_{F} (45,000) of -34 °C and (8) a penetration Hardness, (tenths of mm) at 25°C (77 degrees Fahrenheit) of 3.6.

The Na601 is believed to have a number average molecular weight (Mn) of about 4,600; a weight average molecular weight (Mw) of about 22,400 and a Z average molecular weight (Mz) of about 83,300. The polydisperisity of the Na601 (Mw/Mn) is about 4.87.
where Mn is calculated by the formula:
and Mw is calculated by the formula:
and MZ is calculated by the formula:
where:
- MW =: The various molecular weights of the individual molecules in a sample, and
- n =: The number of molecules in the given sample which have a given molecular weight of MW.

Blending polyolefins with the S-I-S and S-B-S block copolymers followed by meltblowing of the blend has, to date, proved to be unsatisfactory in that the blends appear to be incompatible. However, a good material for blending with the S-I-S block copolymers is poly (alpha-methylstyrene) and a preferred poly (alpha-methylstyrene) may be obtained from Amoco under the trade designation 18-210.

Preferably, the fibrous nonwoven gatherable web 50 portion of the composite nonwoven elastic web 52 formed by the process of the present invention may be formed from any gatherable material which may be formed into a fibrous nonwoven gatherable web 50. For example, the fibrous nonwoven gatherable web 50 could be formed from a blend of a nonelastic material with an elastic material, one or more nonelastic materials or a blend of one or more elastic materials with two or more nonelastic materials. Preferably, the fibrous nonwoven gatherable web 50 is formed from a fiber-forming meltblowable or spunbondable nonelastic gatherable material. Exemplary fiber-forming materials for use in forming the fibrous nonwoven gatherable web are polyester materials, polyolefin materials or blends of one or more polyester materials with one or more polyolefin materials. An exemplary polyester fiber-forming material is polyethylene terephthalate. An exemplary fiber-forming polyolefin material is polypropylene. Preferred polypropylene materials may be obtained under the trade designation PC 973 and PF 301 from the Himont Company.

Typical characteristics of the Himont PC-973 polyproylene stated by Himont are a density of about 0.900 g/cm³, measured in accordance with ASTM D 792; a meltflow rate obtained in accordance with ASTM D 1238, condition L, of 35 g/10 min, tensile of about 29.6 kN/m² (4,300 pounds per square inch (psi)) measured in accordance with ASTM D 638; flex modulus of about 1.25 MN/m² (182,000 psi) measured in accordance with ASTM D 790, B and a Rockwell hardness, R scale, of 93 measured in accordance with ASTM D 785 A. The PC-973 is believed to have a number average molecular weight (Mn) of about 40,100; a weight average molecular weight (Mw) of about 172,000 and a Z average molecular weight of about 674,000. The polydispersity (Mw/Mn) of the PC-973 is about 4.29.

If the gatherable web 50 is to be separated from the elastic web 22 after it has been gathered, it is preferred that the gathered web 50 be capable of substantially returning to its gathered condition upon its separation from the elastic web 22. It is presently believed that, in most embodiments, the gathered condition (e.g., configuration) which the fibrous nonwoven gatherable web 50 exhibits upon its separation from the web 22 will be somewhat longer in the direction of gathering (i.e. machine direction) as compared to the length of the same amount of web 50 when the web 50 is separably joined to the elastic web 22. In other words, the web 50 will extend somewhat in the direction of gathering after its separation from the web 22. Accordingly, the gathered, relaxed, unbiased length of the separated web 50 will be somewhat greater than or equal to the gathered, relaxed, unbiased length of the same amount of the web 50 while it is joined to the elastic web 22.

In one particular embodiment of the present invention the composite nonwoven elastic web 52 is composed of a fibrous nonwoven elastic web 22 which is joined to a gatherable fibrous nonwoven web 50. The composite nonwoven elastic web 52 of this embodiment differs from the composite nonwoven elastic web 52 of the above-described embodiments in that the joining of the two webs 22 and 50 of the composite nonwoven elastic web 52 is achieved without application of heat and/or pressure during the bonding step yet is stronger than the joining achieved by entanglement of the fibers of the nonwoven gatherable web 50 with the fibers of the nonwoven elastic web 22 during formation of the web 50 on the web 22. In this particular embodiment the fibrous nonwoven elastic web 22 is formed from a tacky elastomeric material so that, upon its formation, the fibrous nonwoven elastic web 22 is tacky. The tacky fibrous nonwoven elastic web 22 is formed by meltblowing the web 22 onto the porous collecting screen 14. Alternatively, a tacky nonwoven elastic apertured film (not shown) could be substituted for the tacky fibrous nonwoven elastic web 22. Thereafter, the tacky fibrous nonwoven elastic web 22 is stretched to a stretched length of at least about one and one quarter, that is at least about 125 % of its relaxed, unbiased length by the combined action of the rollers 20 and 26 and 30 and 32 preferably to a length of from about 150 % of the relaxed, unbiased length, to about 700 % or more of the relaxed, unbiased length of the tacky fibrous nonwoven web 22.

After the tacky fibrous nonwoven elastic web 22 has been stretched it is carried by the second porous collecting screen 36 to the nip or gap 42 between the rotating roller 40 and the rotating nip roller 44. While the web 22 is being carried by the second porous collecting screen 36, the fibrous nonwoven gatherable web 50 is formed directly on the upper surface of the tacky web 22 by either a conventional meltblowing or spunbonding process or by any other conventional method which may be utilized to form a fibrous nonwoven gatherable web 50, such as, for example, conventional carding apparatus for forming a carded web. As was the case with the prior discussed embodiments, during formation of the fibrous nonwoven gatherable web 50 on the surface of the web 22 the tacky fibrous nonwoven elastic web 22 is maintained at its stretched, biased length by appropriately adjusting the peripheral surface speed of the rollers 40 and 44 with respect to the peripheral speed of the rollers 30 and 32. As a result of the fact that the fibrous nonwoven elastic web 22 is, upon its formation, tacky, an improved joining (as compared to joining of the two webs solely by entanglement) of the tacky fibrous nonwoven elastic web 22 to the fibrous nonwoven gatherable web 50 is achieved by adhesion of the two webs 20 and 50 to each other during formation of the fibrous nonwoven gatherable web 50 upon the top surface of the fibrous nonwoven elastic web 22. This results in the simultaneous formation and joining of the fibrous nonwoven gatherable web 50 to the fibrous nonwoven elastic web 22. While any tacky elastomeric material may be utilized in forming the tacky fibrous nonwoven elastic web 22 of this embodiment a preferred tacky elastomeric material is an elastomeric A-B-A' block copolymer, where A and A' are each thermoplastic polystyrene endblocks and where B is a polyisoprene midblock. Tri-block copolymer materials of this type are sometimes called S-I-S block copolymers and may be obtained under the trade designation KRATON® D, for example, KRATON® D 1107, KRATON® D 1111, KRATON® D 1112 and KRATON® D 1117, from the Shell Chemical Company. Alternatively, a blend of a S-I-S block copolymer and poly (alpha-methylstyrene) may be utilized.

The materials which may be utilized to form the fibrous nonwoven gatherable web 50 of this embodiment may include any of the materials which were stated above with regard to the fibrous nonwoven gatherable web 50. That is, the fibrous nonwoven gatherable web may be formed from any gatherable material which may be formed into a fibrous nonwoven gatherable web 50. For example, the fibrous nonwoven gatherable web 50 could be formed from a blend of a nonelastic material with an elastic material, one or more nonelastic materials or a blend of one or more elastic materials with two or more nonelastic materials. Preferably, the fibrous nonwoven gatherable web 50 is formed from a fiber-forming meltblowable or spunbondable nonelastic gatherable material. However, the fibrous nonwoven gatherable web 50 may be formed by depositing a carded web on the surface of the fibrous nonwoven elastic web 22 or by any other method which may be utilized to form a fibrous nonwoven gatherable web 50 on the surface of the web 22. Exemplary fiber-forming materials for use in forming the fibrous nonwoven gatherable web 50 are polyester materials, polyolefin materials or blends of one or more polyester materials with one or more polyolefin materials. An exemplary polyester fiber-forming material is polyethylene terephthalate. An exemplary fiber-forming polyolefin material is polypropylene. Preferred polypropylene materials may be obtained from the Himont Company under the trade designations PC 973 and PF 301.

In some situations it may be desirable to incorporate discrete particles of one or more solid materials into one or both of the webs 22 and 50 during formation of the webs 22 and 50. For example, it may be desirable to incorporate one or more fibers such as cotton fibers, wood pulp fibers, polyester fibers or other particulates into one or both of the webs 22 and 50 during their formation. This may be accomplished by utilization of conventional coforming apparatus in conjunction with the meltblowing or spunbonding apparatus 12 and/or 48. Such coforming apparatus is well known to those in the art and is generally illustrated by the apparatus disclosed in U. S. patent 4,100,432 to Anderson.

After the fibrous nonwoven gatherable web 50 has been formed upon and simultaneously joined to the upper surface of the fibrous nonwoven tacky elastic web 22 the composite nonwoven elastic web 52 is passed through the rollers 40 and 44 which, for the reasons stated above, need not be heated or need not apply any excessive pressure to the composite elastic web 52. Thereafter, the stretching and biasing force on the tacky nonwoven elastic web 22 is released so as to relax and contract the composite nonwoven elastic web 52. Because the fibrous nonwoven gatherable web 50 is joined to the surface of the tacky fibrous nonwoven elastic 22 while the tacky fibrous nonwoven elastic web 22 is stretched, relaxing and contraction of the composite nonwoven tacky web 52 results in the fibrous nonwoven gatherable web 50 being carried with, contracted and thereby gathered into a soft batted or matted web 50 which is joined to the surface of the elastic web 22.

### EXAMPLE I

A fibrous nonwoven elastic web which had previously been formed by meltblowing a blend of 60 %, by weight, of an A-B-A' block copolymer having polystyrene A and A' end blocks and a poly (ethylene-butylene) "B" midblock (obtained from the Shell Chemical Company under the trade designation KRATON® GX 1657) and 40 %, by weight, of a polyethylene (obtained from U.S.I. Chemical Company under the trade designation PE Na601) was provided in rolled-up form.

The prior meltblowing of the fibrous nonwoven elastic web was accomplished by extruding the blend of materials through a meltblowing die having thirty extrusion capillaries per lineal inch of die tip. The capillaries each had a diameter of about 0.037 cm (0.0145 inches) and a length of about 0.287 cm (0.113 inches). The blend was extruded through the capillaries at a rate of about 0.52 g per capillary per min at a temperature of about 313°C (595 degrees Fahrenheit). The extrusion pressure exerted upon the blend was measured as 503 N/m² (73 pounds per square inch), gage in the capillaries. The die tip configuration was adjusted so that it was recessed about 0.229 cm (0.090 inches) inwardly from the plane of the external surface of the air plates which form the forming air gaps on either side of the capillaries. The air plates were adjusted so that the two forming air gaps, one on each side of the extrusion capillaries, formed air gaps of about 0.170 cm (0.067 inches). Forming air for meltblowing the blend was supplied to the air gaps at a temperature of about 316°C (600 degrees Fahrenheit) and at a pressure of about 27.6 N/m² (4 pounds per square inch), gage. The meltblown fibers thus formed were blown onto a forming screen which was approximately 38 cm (15 inches) from the die tip.

Later, the thus formed fibrous nonwoven elastic web was unrolled and stretched by applying a tensioning, i.e. biasing, force in the machine direction (MD) and a fibrous nonwoven gatherable web was formed on the surface of the elastic web by meltblowing polypropylene (obtained from the Himont Company under the trade designation PC 973) as microfibers onto the upper surface of the fibrous nonwoven elastic web while the fibrous nonwoven elastic web was maintained at its stretched length.

Meltblowing of the fibrous nonwoven gatherable polypropylene web was accomplished by extruding the polypropylene through a meltblowing die having thirty extrusion capillaries per lineal inch of die tip. The capillaries each had a diameter of about 0.037 cm (0.0145 inches) and a length of about 0.287 cm (0.113 inches). The polypropylene was extruded through the capillaries at a rate of about 0.38 g per capillary per min and at a temperature of about 310°C (590 degrees Fahrenheit). The extrusion pressure exerted upon the polypropylene was measured as 200 N/m² (29 pounds per square inch), gage in the capillaries. The die tip configuration was adjusted so that it was about coplanar with the plane of the external surface of the air plates which form the forming air gaps on either side of the capillaries. The air plates were adjusted so that the two forming air gaps, one on each side of the extrusion capillaries, formed air gaps of about 0.038 cm (0.015 inches). Forming air for meltblowing the polypropylene was supplied to the air gaps at a temperature of about 316°C (600 degrees Fahrenheit) and at a pressure of about 27.6 N/m² (4 pounds per square inch), gage. The meltblown polypropylene microfibers thus formed were meltblown directly onto the upper surface of the fibrous nonwoven elastic web which was located approximately sixteen inches from the die tip. Because of these processing conditions the viscosity of the polypropylene was about 2 Pa s (20 poise) and very fine diameter polypropylene microfibers were formed on the surface of the fibrous nonwoven elastic web.

Next, the tensioning, biasing force was reduced so as to allow the fibrous nonwoven elastic web to retract and for the meltblown polypropylene web to be gathered in the machine direction. The composite nonwoven elastic web which was formed had inter-layer integrity which, apparently, resulted from the entanglement of the individual fibers of the two webs with each other since the webs were not otherwise joined by adhesives or heat-bonding.

Samples of the fibrous nonwoven elastic web, itself, and samples of the composite nonwoven elastic web were then stretched by an Instron tensile tester model 1122 which elongated each sample 100 %, that is twice its unstretched length, and then allowed the sample to return to an unstretched condition. This procedure was then repeated three times and then each sample was elongated to break. Each sample was 5.08 cm (two (2) inches) wide and 12.7 cm (five (5) inches) long and the initial jaw separation on the tester was set at 2.54 cm (one (1) inch). The samples were placed lengthwise in the tester and elongated at a rate of 12.7 cm (five (5) inches) per min. The machine direction data was obtained from samples having a machine direction length of 12.7 cm (five (5) inches) and a transverse direction width of 5.08 cm (two (2) inches). The transverse or cross machine direction measurements were obtained from samples having a length of 12.7 cm (five (5) inches) in the transverse machine direction and a width of 5.08 cm (two (2) inches) in the machine direction. The data which was obtained for the fibrous nonwoven elastic web is tabulated in Table III below and the data which was obtained for the composite elastic web is tabulated in Table IV below.

**TABLE III**

| FIBROUS NONWOVEN ELASTIC WEB | | | | |
|---|---|---|---|---|
| Machine Direction Measurement | | | | |
| Stretched | Stretch Number | Peak TEA* cm/kg (Inch-Pounds) | Peak Load, kg (Pounds) | Peak Elongation, cm (Inches) |
| 100% | #1 Avg** | 10.85 (1.94) | 0.4424 (.9744) | 2.532 (.9968) |
| | Std Dev*** | 2.24 ( .40) | 0.089 (.197) | 0.0022 (.0009) |
| 100% | #2 Avg | 7.65 (1.38) | 0.4224 (.9303) | 2.507 (.9870) |
| | Std Dev | 1.62 ( .29) | 0.085 (.188) | 0.0015 (.0006) |
| 100% | #3 Avg | 7.27 (1.30) | 0.4120 (.9074) | 2.508 (.9873) |
| | Std Dev | 1.57 ( .28) | 0.082 (.181) | 0.0020 (.0008) |
| 100% | #4 Avg | 6.94 (1.24) | 0.4042 (.8903) | 2.508 (.9873) |
| | Std Dev | 1.40 ( .25) | 0.081 (.178) | 0.0013 (.0005) |
| To break | #5 Avg | 56.40 (10.08) | 0.6578 (1.4488) | 7.974 (3.1394) |
| | Std Dev | 17.57 (3.14) | 0.1354 (.2982) | 1.316 (.5181) |

| Transverse Direction Measurements | | | | |
|---|---|---|---|---|
| Elongation Stretched | Stretch Number | Peak TEA* cm/kg (Inch-Pounds) | Peak Load, kg (Pounds) | Peak Elongation, cm (Inches) |
| 100% | #1 Avg** | 8.39 (1.50) | 0.3546 (.7811) | 2.533 (.9974) |
| | Std Dev*** | 0.67 ( .12) | 0.0269 (.0593) | 0.0043 (.0017) |
| 100% | #2 Avg | 6.04 (1.08) | 0.3386 (.7459) | 2.506 (.9866) |
| | Std Dev | 0.45 ( .08) | 0.0258 (.0568) | 0.0023 (.0009) |
| 100% | #3 Avg | 5.65 (1.01) | 0.3296 (.7261) | 2.507 (.9870) |
| | Std Dev | 0.42 ( .07) | 0.0246 (.0542) | 0.0018 (.0007) |
| 100% | #4 Avg | 5.37 ( .96) | 0.3224 (.7107) | 2.505 (.9863) |
| | Std Dev | 0.42 ( .07) | 0.0242 (.0533) | 0.0020 (.0008) |
| To break | #5 Avg | 58.24 (10.41) | 0.5879 (1.295) | 9.256 (3.644) |
| | Std Dev | 6.94 (1.24) | 0.043 (.095) | 0.681 (.268) |

**TABLE IV**

| COMPOSITE NONWOVEN ELASTIC WEB | | | | |
|---|---|---|---|---|
| Machine Direction Measurement | | | | |
| Elongation Stretched | Stretch Number | Peak TEA* cm/kg (Inch-Pounds) | Peak Load kg (Pounds) | Peak Elongation, cm (Inches) |
| 100% | #1 Avg** | 11.41 (2.04) | 0.5723 (1.2606) | 2.444 (.9976) |
| | Std Dev*** | 0.95 ( .17) | 0.0360 (0.0793) | 0.0023 (.0009) |
| 100% | #2 Avg | 7.67 (1.37) | 0.5473 (1.2056) | 2.506 (.9866) |
| | Std Dev | 0.67 ( .12) | 0.0368 (.0810) | 0.0030 (.0012) |
| 100% | #3 Avg | 7.22 (1.29) | 0.5356 (1.1798) | 2.508 (.9874) |
| | Std Dev | 0.62 ( .11) | 0.0351 (.0773) | 0.0028 (.0011) |
| 100% | #4 Avg | 6.94 (1.24) | 0.5285 (1.161) | 2.509 (.9876) |
| | Std Dev | 0.62 ( .11) | 0.0360 (.0792) | 0.0030 (.0012) |
| To break | #5 Avg | 54.00 (9.65) | 1.1411 (2.5134) | 5.794 (2.281) |
| | Std Dev | 10.46 (1.87) | 0.0753 (.1659) | 0.5697 (.2243) |

| Transverse Direction Measurements | | | | |
|---|---|---|---|---|
| Elongation Stretched | Stretch Number | Peak TEA* cm/kg (Inch-Pounds) | Peak Load kg (Pounds) | Peak Elongation cm (Inches) |
| 100% | #1 Avg** | 12.76 (2.28) | 0.5798 (1.277) | 2.288 (.9009) |
| | Std Dev*** | 2.69 ( .48) | 0.0723 (.1593) | 0.2286 (.0900) |
| 100% | #2 Avg | 3.92 ( .70) | 0.4890 (1.077) | 2.503 (.9853) |
| | Std Dev | 0.50 ( .09) | 0.1002 (.2206) | 0.0005 (.0002) |
| 100% | #3 Avg | 3.25 ( .58) | 0.4640 (1.022) | 2.508 (.9874) |
| | Std Dev | 0.45 ( .08) | 0.0971 (.2139) | 0.0033 (.0013) |
| 100% | #4 Avg | 2.97 ( .53) | 0.4470 (.9846) | 2.508 (.9873) |
| | Std Dev | 0.45 ( .08) | 0.0975 (.2148) | 0.0030 (.0012) |
| To break | #5 Avg**** | 4.92 ( .88) | 0.5262 (1.159) | 2.760 (1.0865) |
| | Std Dev | 1.17 ( .21) | 0.1008 (.2220) | 0.0305 (.0120) |

Tables III and IV disclose the total energy absorbed, in cm/kg (inch-pounds), the peak (maximum) load, in kg (pounds), encountered during each repetition and the amount of each peak (maximum) elongation, in cm (inches) in stretching the samples in each repetition of the 100 % elongation procedure and in elongating the sample to break. It can be seen that the total energy required to stretch the sample 100 % in the machine direction at the peak load encountered in such stretching is about the same for the fibrous nonwoven elastic web and the composite nonwoven elastic web. This is to be expected since the meltblown polypropylene web is gathered in the machine direction and generally requires little energy to be elongated in the machine direction. Upon elongation to break, the peak load for the composite nonwoven elastic web increased over 70 % indicating that the meltblown polypropylene web was contributing strength to the strength of the composite nonwoven elastic web.

In the transverse machine direction (TD), where the meltblown polypropylene is not gathered, the peak load for the initial stretch of the composite nonwoven elastic web is over 60 % greater than the peak load for the fibrous nonwoven elastic web. This indicates that the meltblown polypropylene web contributes to the strength of the composite nonwoven elastic web even at low elongations. Additionally, the peak total energy absorbed for the composite nonwoven elastic web represents a 50 % increase over that of the fibrous nonwoven elastic web for the first stretch and then actually decreases on subsequent stretchings. This indicates that the meltblown polypropylene web was substantially ruptured (torn) during the first stretch and is no longer contributing to total energy of the composite web.

It was observed that the "breathability" of the composite nonwoven elastic web was still good as compared to the "breathability" of the fibrous nonwoven elastic web. Additionally, because of the thin web of meltblown polypropylene microfibers which have been applied to the surface of the fibrous nonwoven elastic web the composite web was more water repellent due to the water repellent characteristics of polypropylene. Moreover, application of the thin web of meltblown microfibers to the surface of the meltblown nonwoven elastic web changed the rubbery feel of the fibrous nonwoven elastic web to a soft, desirable feeling.

### EXAMPLE II

A fibrous nonwoven web which had previously been formed by meltblowing a blend of 60%, by weight, of an A-B-A' block copolymer having polystyrene "A" and "A'" endblocks and a poly (ethylene-butylene) "B" midblock (obtained from the Shell Chemical Company under the trade designation KRATON® GX 1657) and 40% by weight, of a polyethylene (obtained from U.S.I. under the trade designation PE Na 601) was provided in rolled-up form.

The prior meltblowing of the fibrous nonwoven elastic web was accomplished by extruding the blend of materials through a meltblowing die having thirty extrusion capillaries per lineal 2.54 cm (inch) of die tip. The capillaries had a diameter of about 0.0368 cm (0.0145 inches) and a length of about 0.287 cm (0.113 inches). The blend was extruded through the capillaries at a rate of about 0.50 g per capillary per min at a temperature of about 299°C (570 degrees Fahrenheit). The extrusion pressure exerted upon the blend was measured as 0.99 kN/m² (144 pounds per square inch), gage in the capillaries. However, it is presently believed that this measurement was inaccurate due to a faulty pressure probe. The die tip configuration was adjusted so that it was recessed about 0.279 cm (0.110 inches) inwardly from the plane of the external surface of the air plates which form the forming air gaps on either side of the capillaries. The air plates were adjusted so that the two forming air gaps, one on each side of the extrusion capillaries, formed gaps of about 0.279 cm (0.110 inches). Forming air for meltblowing the blend was supplied to the air gaps at a temperature of about 323°C (614 degrees Fahrenheit) and at a pressure of about 27.6 N/m² (4 pounds per square inch), gage. The meltblown microfibers were formed onto a forming screen which is believed to have been about 40.64 cm (16 inches) from the die tip. However, measurement of this distance was not actually taken.

Later, the thus formed fibrous nonwoven elastic web was unrolled and stretched by applying a tensioning, i.e. biasing, force in the machine direction (MD) and a fibrous nonwoven gatherable web was formed on the surface of the elastic web by meltblowing polypropylene (obtained from the Himot Company under the trade designation PF 301) as microfibers on to the upper surface of the fibrous nonwoven elastic web while the fibrous nonwoven elastic web was maintained at its stretched length.

Meltblowing of the fibrous nonwoven polypropylene gatherable web was accomplished by extruding the polypropylene through a meltblowing die having thirty extrusion capillaries per lineal 2.54 cm (inch) of die tip. The capillaries each had a diameter of about 0.0368 cm (0.0145 inches) and a length of about 0.287 cm (0.113 inches). The polypropylene was extruded through the capillaries at a rate of about 0.75 g per capillary per min at a temperature of about 310°C (590 degrees Fahrenheit). The extrusion pressure exerted upon the polypropylene was measured as about 1.28 kN/m² (186 pounds per square inch), gage in the capillaries. The die tip configuration was adjusted so that it extended about 0.025 cm (0.010 inches) beyond the plane of the external surface of the air plates which form the forming air gaps on either side of the capillaries. The air plates were adjusted so that the two forming air gaps, one on each side of the extrusion capillaries, formed air gaps of about 0.046 cm (0.018 inches). Forming air for meltblowing the polypropylene was supplied to the air gaps at a temperature of about 316°C (600 degrees Fahrenheit) and at a pressure of about 14 N/m² (2 pounds per square inch), gage. The distance between the die tip and the surface of the fibrous nonwoven elastic web upon which the gatherable polypropylene web was formed was about 25.4 cm (10 inches). Because of these processing conditions, the viscosity of the polypropylene was about 12.4 Pa s (124 poise) and larger diameter meltblown polypropylene microfibers were formed on the surface of the stretched fibrous nonwoven elastic web.

Next, the tensioning, biasing force was reduced so as to allow the fibrous nonwoven elastic web to contract and for the meltblown polypropylene web to be gathered in the machine direction. The composite nonwoven elastic web which was formed had inter-layer integrity which, apparently, resulted from the entanglement of the individual fibers of the two webs with each other since the webs were not otherwise joined by adhesives or heat-bonding.

Samples of this fibrous nonwoven elastic web, itself, and samples of the composite nonwoven elastic web were then stretched by an Instron tensile tester model 1122 which elongated each sample 100 %, that is to twice its unstretched length, and then allowed the sample to return to an unstretched condition. This procedure was then repeated 3 times and then each sample was elongated to break. Each sample was 5.1 cm (2 inches) wide by 12.7 cm (5 inches) long and the initial jaw separation on the tester was set at 2.54 cm (1 inch). The samples were placed lengthwise in the tester and elongated at a rate of 12.7 cm (5 inches) per min. The machine direction data was obtained from samples having a machine direction length of 12.7 cm (5 inches) and a transverse direction width of 5.1 cm (2 inches). The transverse or cross machine direction measurements were obtained from samples having a length of 12.7 cm (5 inches) in the transverse direction and a width of 5.1 cm (2 inches) in the machine direction. The data which was obtained for the composite nonwoven elastic web formed by example 2 is tabulated in Table V below.

Table V, below, illustrates that the, 100 %, elongations required little energy or load in the machine direction while the total energy absorbed increased about 7 times and the peak load increased about 3 times when the composite was stretched to break in the machine direction. In the transverse direction, where the meltblown was not gathered, the initial, 100 % elongation absorbed about 3.5 times as much total energy as the total energy absorbed to break and about 4 to 5 times as much energy as any of the subsequent, 100 % stretchings. Further, the peak load for the first stretching in the transverse direction was about 40 % higher than the peak load for any subsequent stretching in the transverse direction, including stretching to break.

**TABLE V**

| COMPOSITE NONWOVEN ELASTIC WEB | | | | |
|---|---|---|---|---|
| Machine Direction Measurement | | | | |
| Elongation Stretched | Stretch Number | Peak TEA* cm/kg (Inch-Pounds) | Peak Load kg (Pounds) | Peak Elongation cm (Inches) |
| 100% | #1 Avg** | 5.31 ( .95) | 0.3499 (.7708) | 2.5344 (.9978) |
| | Std Dev*** | 1.57 ( .28) | 0.0790 (.1742) | 0.0041 (.0016) |
| 100% | #2 Avg | 4.20 ( .75) | 0.3354 (.7388) | 2.5070 (.9870) |
| | Std Dev | 1.29 ( .23) | 0.0760 (.1675) | 0.0038 (.0015) |
| 100% | #3 Avg | 3.97 ( .71) | 0.3271 (.7204) | 25.0546 (.9864) |
| | Std Dev | 1.23 ( .22) | 0.0743 (.1636) | 0.0025 (.0010) |
| 100% | #4 Avg | 3.80 ( .68) | 0.3216 (.7083) | 2.5044 (.9860) |
| | Std Dev | 1.23 ( .22) | 0.0740 (.1631) | 0.0028 (.0011) |
| At break | #5 Avg | 32.17 (5.75) | 0.8962 (1.974) | 5.138 (2.023) |
| | Std Dev | 7.61 (1.36) | 0.1106 (.2437) | 0.5174 (.2037) |

| Transverse Direction Measurements | | | | |
|---|---|---|---|---|
| Elongation Stretched | Stretch Number | Peak TEA* cm/kg (Inch-Pounds) | Peak Load kg (Pounds) | Peak Elongation cm (Inches) |
| 100% | #1 Avg** | 17.23 (3.08) | 0.9271 (2.042) | 1.9124 (.7529) |
| | Std Dev*** | 4.31 ( .77) | 0.1059 (.2333) | 0.2319 (.0913) |
| 100% | #2 Avg | 4.64 ( .83) | 0.6456 (1.422) | 2.5085 (.9876) |
| | Std Dev | 0.45 ( .08) | 0.1397 (.3076) | 0.0025 (.0010) |
| 100% | #3 Avg | 4.03 ( .72) | 0.6085 (1.3403) | 2.507 (.9870) |
| | Std Dev | 0.45 ( .08) | 0.1319 (.2905) | 0.0023 (.0009) |
| 100% | #4 Avg | 3.64 ( .65) | 0.5816 (1.281) | 2.5090 (.9878) |
| | Std Dev | 0.39 ( .07) | 0.1244 (.2740) | 0.0030 (.0012) |
| At break | #5 Avg | 4.76 ( .85) | 0.6002 (1.322) | 2.6721 (1.052) |
| | Std Dev | 0.39 ( .07) | 0.1135 (.2500) | 0.1133 (.0446) |

### NOTES FOR TABLES III, IV AND V

- *: = Total Energy Absorbed
- **: = Average
- ***: = Standard Deviation
- ****: = Average of two measurements. The third measurement obtained values of 13.294 (2.376) for Peak TEA, 0.559 (1.232) for Peak Load and 14.247 (5.609) Peak Elongation. These values are believed to be incorrect since they are so abberant from the other values obtained by the other two measurements.

Unless otherwise specifically noted the data reported in tables III, IV and V (above) represent an average value which was obtained by taking five individual measurements for each machine direction measurement and three individual measurements for each transverse direction measurement.

The basis weight of the meltblown fibrous nonwoven elastic web utilized for example I was 67.3 g/m² and the basis weight of the meltblown gatherable polypropylene web which was formed on the surface of the fibrous nonwoven elastic web of example I was measured as being 12.2 g/m². The degree of relaxation or contraction of the composite nonwoven elastic web of example I was about 54 %. This degree of relaxation of the composite was determined by taking a sample of the composite having a relaxed length of about 10.16 cm (4.0 inches) in the machine direction and elongating the sample, in the machine direction, until resistance to the elongation by the gathered polypropylene web was encountered. That is, just until the gathers in the polypropylene web were removed. At this point the 10.16 cm (4.0 inch) sample had been stretched to about 22.23 cm (8.75 inches) in the machine direction.

The basis weight of the fibrous nonwoven elastic web utilized in example II was about 66.2 g/m² and the basis weight of the fibrous nonwoven gatherable polypropylene web meltblown onto the surface of the elastic web in example II was measured at about 21.4 g/m². The degree of relaxation or contracting of the composite nonwoven elastic web of example II was determined to be about 42 %. This degree of relaxation was determined by taking a sample of the composite having a relaxed length of about 30.48 cm (12 inches) in the machine direction and elongating the sample, in the machine direction, until resistance to the elongation by the gathered polypropylene web was encountered. That is, just until the gathers in the polypropylene web were removed. At this point the 30.48 cm (12 inch) sample had been stretched to about 52.58 cm (20.7 inches).

Upon observation of the relaxed, contracted composite nonwoven elastic web it was seen that the meltblown polypropylene web presented a creped, gathered, appearance with the lines of creping or gathering being generally transverse to the direction in which the fibrous nonwoven elastic web was stretched during formation of the meltblown polypropylene web on the surface of the fibrous nonwoven elastic web (i.e. transverse to the machine direction). Interestingly, it was also observed that the fibrous nonwoven elastic web of the contracted and relaxed composite nonwoven elastic web exhibited lines of creping or gathering which were generally parallel to the direction of stretching of the fibrous nonwoven elastic web during formation of the meltblown polypropylene included on the surface thereof (i.e. the lines of creping or gathering of the fibrous nonwoven elastic web were generally parallel to the machine direction). Accordingly, the two webbed composite included webs having transposed lines of gathering or creping which generally crossed each other generally at right angles. Formation of the lines of gathering or creping in the fibrous nonwoven gatherable polypropylene web would be expected in view of the gathering of that web in the machine direction. However, formation of lines of gathering or creping in the fibrous nonwoven elastic web and, in particular, formation of lines of gathering or creping in the fibrous nonwoven elastic which are generally at right angles with the lines gathering or creping of the fibrous nonwoven gatherable polypropylene webs was unexpected.

A portion of the composite nonwoven elastic web having an approximate machine direction (MD) length of about 14.9 cm (5 and 7/8 inches) and an approximate transverse direction (TD) dimension of about 11.4 cm (4-1/2 inches) was cut off of the composite nonwoven elastic web and the gathered fibrous nonwoven meltblown polypropylene web was separated from the fibrous nonwoven elastic web. After the gathered fibrous nonwoven meltblown polypropylene web had been separated from the fibrous nonwoven elastic web it was observed that the gathered fibrous nonwoven meltblown polypropylene web assumed a relaxed machine direction dimension of about 17.78 cm (7 inches) and retained its cross-direction dimension of about 11.43 cm (4-1/2 inches). Importantly, the fibrous nonwoven gathered web substantially retained its creped or gathered configuration in the machine direction. Moreover, the separated gathered polypropylene web could be elongated in the machine direction upon application of a tensioning and biasing force in the machine direction and would, upon removal of the tensioning and biasing force, return, that is, contract, substantially to its relaxed and unbiased and untensioned gathered dimension 17.78 by 11.43 cm (7 inches by 4-1/2 inches). For example, upon elongation of the 17.78 by 11.43 cm (7 inch by 4-1/2 inch) sample of gathered fibrous nonwoven polypropylene web in the machine direction (MD) to an extent where the gathers had been substantially straightened out, the sample was measured and found to have a machine direction (MD) length of about 24.13 cm (9-1/2 inches) and a transverse direction (TD) dimension of about 11.43 cm (4-1/2 inches). When the elongating, biasing force was removed from the sample it returned to a machine direction (MD) dimension of just over seven inches and a transverse direction (TD) dimension of about 11.43 cm (4-1/2 inches) within one minute. Upon repetition of the elongation procedure, the sample assumed a machine direction (MD) dimension of about 24.13 cm (9-1/2 inches) and a transverse direction (TD) dimension of about 11.43 cm (4-1/2 inches). Upon termination of the second elongating and stretching force, the polypropylene web assumed a machine direction (MD) dimension of about 17.94 cm (7-1/16 inches) and a transverse direction (TD) dimension of about 11.43 cm (4-1/2 inches) within one minute. This result was unexpected since the PF 301 polypropylene was not believed to possess elastic properties.

Other variations of the present process and the product formed by the process are possible. For example, two or more fibrous nonwoven gatherable webs 50 could be bonded one on top of another in stacked configuration to give the fibrous nonwoven gatherable web 50 additional thickness. Additionally, a fibrous nonwoven gatherable web 50 could be joined, either separably or otherwise as discussed herein, to both surfaces of the fibrous nonwoven elastic web 22 to form a composite nonwoven elastic web having the following three web sequence: fibrous nonwoven gatherable web/fibrous nonwoven elastic web/fibrous nonwoven gatherable web.

The three web sequence where the fibrous nonwoven elastic web is sandwiched between two fibrous nonwoven gatherable webs is especially preferred where the fibrous nonwoven elastic web 22 is formed from a tacky elastomeric material as described above because sandwiching of the tacky elastic web 22 between the two webs prevents the tacky web 22 from adhering to other portions of the web 52 upon rolling-up of the web 52 for storage. The three web material could be formed by the process which is illustrated schematically in figure 3. This process is identical to the process schematically illustrated in figure 1 until the two layered composite nonwoven elastic web 52 exits rollers 40 and 42. Thereafter, instead of proceding to the nip or gap 54 between the roller 56 and 58, the composite web 52 passes through the nip or gap 78 between a rotating roller 80 and a rotating nip roller 82. The composite web 52 is then carried by a third porous collecting screen 84 to the nip or gap 86 between a rotating nip roller 88 and a rotating roller 74. The porous collecting screen 68 moves about and is driven by the rollers 80 and 84 in the direction indicated by the arrows 92 in figure 3. Rotation of the rollers 80, 82, 88 and 90 is adjusted so that the peripheral surface speed of the rollers 80, 82, 88 and 90 is the same as the peripheral surface speed of the rollers 40 and 44. Accordingly, the fibrous nonwoven elastic web 22 is maintained at its stretched, biased length as it is carried by the porous collecting screen 84.

While the composite nonwoven elastic web 52 is being carried by the porous collecting screen 84, a conventional meltblowing die 94 (if desired, a conventional spunbonding die or carding apparatus can be utilized) forms a second nonwoven gatherable web 96 on the other surface of the stretched fibrous nonwoven elastic web 22 by meltblowing microfibers 98 directly onto the stretched upper surface of the nonwoven elastic web 22. The materials which may be utilized to form the second gatherable web 96 may include any of the materials which were stated above as being utilizable to form the first fibrous nonwoven gatherable web 50. Particulate materials may also be incorporated within the web 96 as was stated above with regard to the webs 22 and 50. Thereafter, the second fibrous nonwoven gatherable web 96 may be heat-bonded to the fibrous nonwoven elastic web 22 by the action of rollers 88 and 90 which are essentially equivalent to rollers 40, 44. The heat-bonding of the second fibrous nonwoven gatherable web 96 to the fibrous nonwoven elastic web 22 can be carried out within the same temperature ranges and within the same pressure ranges as were stated above with regard to the heat-bonding of the first fibrous nonwoven gatherable web 50 to the fibrous nonwoven elastic web 22. If desired, conventional sonic bonding techniques (not shown) may be substituted for the heat-bonding step. Alternatively, if the fibrous nonwoven elastic web 22 is tacky, as described above, heat bonding of the fibrous nonwoven gatherable web 96 to the fibrous nonwoven elastic web will not be required since the second fibrous nonwoven gatherable web 96 will be simultaneously formed upon and joined to the surface of the fibrous nonwoven elastic web 22.

In another embodiment, if separation of the gatherable web 96 from the elastic web 22 will be effected at a later step, the second fibrous nonwoven gatherable web 96 may be separably joined to the surface of the fibrous nonwoven elastic web 22 by entanglement of the individual fibers of the web 96 with the individual fibers of the web 22 during formation of the web 96 on the surface of the web 22. In this embodiment the fibrous nonwoven gatherable web 96 is simultaneously formed upon and joined to the fibrous nonwoven elastic web 22.

In any of these embodiments improved joining of the webs 50 and 96 to the web 22 can be effected by application of a coating of an adhesive material to the surface of the elastic web 22 prior to formation of the webs 50 and 96 upon the stretched surface of the web 22. Application of such an adhesive coating to the surface of web 22 may be conventionally readily effected by the nip rollers 32 and 82. For example, the adhesive material could be conventionally applied to the surface of the rollers 32 and 82 so that the rollers 32 and 82 would transfer the adhesive onto the surface of the web 22 as the web 22 passes through the nips 28 and 78. Alternatively, the adhesive may be applied onto the surface of the web 22 in a configuration of spots.

After joining of the gatherable web 96 to the elastic web 22 has been achieved, the biasing force on the web 22 is relaxed by passing the three webbed composite 100 through the nip or gap 102 between two rotating nip rollers 104 and 106. Rotation of the rollers 104 and 106 is adjusted so that the peripheral surface speed of the rollers 104 and 106 allows the composite web 100 to relax and, as a result of its elastic properties, to contract to its relaxed, unbiased length. The relaxing and contracting of the web 100 to its relaxed, unbiased length results in both of the fibrous nonwoven gatherable webs 50 and 96 being gathered by the relaxing and contracting of the fibrous nonwoven elastic web 22. Lastly, the composite web 100 can be rolled up and stored as is illustrated at 108. Since the tacky elastic web 22 is sandwiched between the webs 50 and 96 it will not adhere to other portions of the composite web 100 during storage. This material may be utilized to form a variety of products, such as, for example, diaper products.

It should be recognized that the three webbed composite 100 discussed above with respect to a tacky nonwoven elastic web 22 could be formed without using a tacky material to form the web 22. In this case, the other methods of joining, for example, fibrous entanglement, heat-bonding or sonic bonding, the web 96 to the web 22 would have to be utilized.

Another variation of the present invention would involve gathering of one or more of the gatherable webs 50 and 96 in the transverse machine direction (TD) as opposed to the machine direction (MD) as illustrated in the figures. If gathering of the gatherable webs 50 and/or 96 in the transverse machine direction (TD) is desired, additional arrangements for stretching and allowing contraction of the elastic web 22 in the transverse direction would be utilized. For example, Figure 4 illustrates another embodiment of the present invention which avoids the requirement of forming the gathered nonwoven elastic web 50 of the embodiment of Figure 1 on the stretched, extended surface of the nonwoven elastic web 22. In the embodiment of Figure 4 the gathered nonwoven elastic web 50 is formed directly on the surface of a porous forming screen 110 which, itself, is extendable and retractable in the machine direction of movement as is indicated by the arrow 112. For example, the extendable and retractable porous collecting screen 110 could be formed from a continuous web of the nonwoven elastic web 22. Alternatively, the extendable and retractable porous collecting screen 110 could be formed from a wire mesh screen 114 which is generally illustrated in Figure 5. The wire mesh screen 114 could be formed from a plurality of substantially parallel springs 116 coiled and extending in the machine direction (MD) with the springs 116 being connected to each other in the transverse machine direction (TD) by a plurality of fine, generally parallel wires 118 extending in the transverse machine direction (TD). The transverse direction wires 118 may be arranged very closely to each other so that, when the wire mesh screen 114 is in an unbiased, retracted or contracted configuration, the transverse direction wires 118 contact each other. Upon application of a tensioning or biasing force in the machine direction, the coiled springs 116 will extend, that is, stretch, in the machine direction and the fine transverse direction wires 118 will separate from each other to form the porous collecting surface 110. This biased, stretched, extended configuration is generally illustrated in Figure 6.

Alternatively, the wire mesh screen 114 could be formed by a plurality of substantially parallel springs coiled and extending in the transverse machine direction (TD) with the springs being connected to each other in the machine direction (MD) by a plurality of fine, generally parallel wires extending in the machine direction (MD). This configuration would be illustrated upon rotating Figures 5 and 6 90° and results in a configuration by which the gatherable web 96 could be gathered in the transverse machine direction (TD) as opposed to the machine direction (MD) as is illustrated in the figures. If gathering of the gatherable web 96 in the transverse direction is desired additional conventional arrangements (not shown) for extending and contracting the screen 114 in the transverse direction would replace the arrangement illustrated in the figures for extending and contracting the screen 114 in the machine direction (MD).

Returning to Figure 4 it can be seen that movement of the extendable and retractable porous collecting screen 110 in the machine direction 112 is accomplished by the screen 110 being driven by rollers 120 and 122 which are, in turn, driven by conventional drive mechanism (not shown). Also not shown for purposes of clarity is a conventional vacuum box located between the rollers 120 and 122 and beneath the lower surface of the upper portion of the screen 110. The vacuum box assists in the retention of the web 22 on the upper surface of the screen 110. The extendable and contractable porous collecting screen 110 passes through the nip 124 between a pair of rotating nip rollers 126 and 128. The nip 124 is adjusted so that the rollers 126 and 128 firmly engage the extendable and retractable or contractable porous collecting screen 110 without adversely affecting the screen 110. Rotation of the rollers 126 and 128 is adjusted so that the peripheral surface speed of the rollers 126 and 128 is substantially the same as the peripheral surface speed of the rollers 120 and 122. The extendable and retractable or contractable porous collecting screen 110 also passes through the nip 130 between another pair of rotating nip rollers 132 and 134 with the nip 130 being adjusted so that the rollers 132 and 134 firmly engage the porous collecting screen 110 without adversely affecting the porous collecting screen 110. The rotation of the rollers 132 and 134 is adjusted so that the peripheral surface speed of the rollers 132 and 134 is greater than the peripheral surface speed of the rollers 120 and 122. As a result of the increase in the peripheral surface speed of the rollers 132 and 134 with respect to the peripheral surface speed of the rollers 120 and 122 a longitudinal or machine direction (MD) biasing and extending force is placed on the extendable and contractable porous collecting screen 110 and the screen 110 is extended to an extended, biased length in the longitudinal direction in the area 136. The degree of extension of the porous collecting screen 110 which occurs in the area 136 between the rollers 126 and 128 and the rollers 132 and 134 may be varied, for example, by varying the peripheral surface speed of the rollers 132 and 134 with respect to the peripheral surface speed of the rollers 126 and 128. For example, if the peripheral surface speed of the rollers 132 and 134 is about twice that of the rollers 126 and 128, the extendable and retractable porous collecting screen 110 will be extended to an extended, biased length of substantially about twice, that is, about 200 %, of its retracted, unbiased length. The extendible and retractable porous collecting screen 110 is extended, in the area 136, to a length which is at least about 125 % of its contracted, unbiased and unextended length to about 700 or more % of the retracted, unbiased and unextended length of the porous collecting surface 110. In particular, it is preferred for the screen 110 to be extended to an extended length, in the area 136, of from at least about 150 % of its retracted, unbiased and unextended length.

While the extendable and retractable porous collecting screen 110 is in the extended configuration in the area 136, meltblown microfibers 138, which are formed by a conventional meltblowing die 140 are meltblown onto the extended surface of the porous collecting screen 110. As the meltblown microfibers 138 are deposited upon the extended porous collecting screen 110 they entangle and cohere to form a cohesive fibrous nonwoven gatherable web 96. The entangled cohesive fibrous nonwoven gatherable web 96 is carried by the porous collecting screen 110 through the nip 130 and on to a nip 142 formed between the rotating roller 120 and a rotating nip roller 144. The peripheral surface speed of the rotating nip roller 144 is adjusted so that it is substantially the same as the peripheral surface speed of the rotating roller 120 and the rollers 122 and 126 and 128. Because the peripheral surface speed of the rollers 144 and 120 is substantially the same as the peripheral surface speed of the rollers 122 and 126 and 128 the extending force is removed from the extended porous collecting screen 110 and the screen 110 is retracted, that is allowed to contract, as a result of its contractable properties, to its contracted, unbiased length. The relaxing and contracting of the porous collecting screen 110 to its contracted, unbiased length results in the fibrous nonwoven gatherable web 96, which was formed on the surface of the screen 110 while the screen 110 was being maintained in its extended configuration, being carried along with, and retracted and thus gathered upon the upper surface of the retracting porous collecting screen 110. The gathering of the fibrous nonwoven gatherable web 96, accordingly, occurs in the area 146 between the pairs of rollers 132 and 134 and 120 and 144.

After retracting and contracting of the porous collecting screen 110, the fibrous nonwoven gatherable web 96 may be rolled up on a supply roller 148 for storage and shipment. For the reasons stated earlier the rate of rotation of the supply roller 148 should be controlled so that the gathered fibrous nonwoven 96 is stored in substantially an untensioned state. This may be accomplished by adjusting the rate of rotation of the roller 148 so that the peripheral surface speed of the roller 148 is substantially equal to or just slightly greater than the peripheral surface speed of the rollers 120 and 144.

In the event that a three layer composite web is formed, as illustrated in Figure 3, it may be desirable to separate the two outer gathered nonwoven webs from the elastic nonwoven web. If this is the case the fibrous nonwoven gathered webs 50 and 96 are separated from the fibrous nonwoven elastic web 22 by passing the web 50 through the nip 150 between two rotating nip rollers 152 and 154 and passing the web 96 through the nip 156 between two rotating nip rollers 158 and 160. The webs 50 and 96 are then wound-up for storage and later used on their respective storage rolls 162 and 164. For the reasons stated earlier, care should be exercised in winding-up the gathered nonwoven webs 50 and 96 to assure that the webs 50 and 96 are stored in an untensioned or substantially untensioned fashion on the rolls 162 and 164. This can be effected by rotating the rolls 162 and 164 so that the peripheral surface speed of the roller 162 is equal to or just slightly greater than the peripheral surface speed of the rolls 152 and 154 and that the peripheral surface speed of the roller 164 is equal to or just slightly greater than the peripheral surface speed of the rollers 158 and 160. After separation of the webs 50 and 96 the fibrous nonwoven elastic web 22 passes through the nip 166 between the two rotating nip rollers 168 and 170 and is wound up on a storage roller 172.

While the specific examples discussed herein have usually stated that the fibrous nonwoven gatherable webs 50 and 96 were formed by utilization of a conventional meltblowing die and meltblowing processes, conventional spunbonding dies and spundbonding processes may be substituted for the meltblowing dies and processes and the scope of the present invention is intended to include materials formed by the substitution of spunbonding dies and processes or any other apparatus and process for forming a nonwoven gatherable web for the meltblowing dies and processes 48 and 94. In the event that spunbonding dies and processes were substituted for either or both of the meltblowing dies or processes 48 and 94 joining of the gatherable web(s) 50 and, if applicable 96, to the fibrous nonwoven elastic web 22 should be effected, as stated above, by inter-web adhesion (if a tacky elastomeric material is utilized to form the web 22), by heat-bonding or sonic bonding and/or by application of an adhesive to the surface(s) of the web 22 prior to formation of the web(s) 50 and 96 thereon. These methods of joining should be utilized with spunbonded gatherable web since the fibers of spunbonded gatherable webs do not readily entangle with the fibers of the web 22. If the joining of one or more of the webs 50 and 96 to the web 22 is to be effected by heat-bonding (whether the webs 50 and 96 are spun bonded, meltblown or formed by other processes) care should be taken to allow the web 22 to relax and contract to substantially an untensioned, unbiased condition or configuration as soon as is practical after the heat-bonding step has occurred because it is believed that the nonwoven elastic web 22 will lose its elasticity if it is maintained above its softening for any significant period of time. This loss of elasticity may result from the cooling elastic web 22 "setting" while in the stretched configuration if it is maintained in the stretched configuration for a significant period of time after heat-bonding.

## Claims

1. A process for producing a composite nonwoven elastic web comprising a nonwoven elastic web joined to a fibrous nonwoven gathered web, comprising the step of:
(a) providing a nonwoven elastic web,
**characterized in that** it further comprises the steps of
(b) stretching said nonwoven elastic web from at least about 125% of the relaxed length of the nonwoven elastic web to about 700% of the relaxed length of the nonwoven elastic web;
(c) forming a fibrous nonwoven gatherable web directly upon a surface of the stretched nonwoven elastic web and joining the stretched fibrous nonwoven gatherable web to the stretched nonwoven elastic web so as to form a composite nonwoven elastic web; and
(d) relaxing the composite nonwoven elastic web to gather the fibrous nonwoven gatherable web.

2. The process according to claim 1, **characterized in that** the nonwoven elastic web is a tacky nonwoven elastic web and the composite nonwoven elastic web is formed by forming a fibrous nonwoven gatherable web directly upon a surface of the stretched nonwoven elastic web and simultaneously joining said nonwoven elastic web to the surface of the stretched nonwoven elastic web whereby joining of the tacky nonwoven elastic web to the fibrous nonwoven gatherable web is achieved by adhesion of the two webs to each other during formation of the fibrous nonwoven gatherable web on the surface of the stretched fibrous nonwoven elastic web.

3. The process according to claim 1 **characterized in that** the composite nonwoven elastic web is formed by forming a fibrous nonwoven gatherable web directly upon a surface of the stretched nonwoven elastic web and simultaneously joining the fibrous nonwoven gatherable web to the surface of the stretched nonwoven elastic web whereby joining of the nonwoven elastic web to the fibrous nonwoven gatherable web is achieved by entanglement of the individual fibers of the fibrous nonwoven gatherable web with the nonwoven elastic web during formation of the fibrous nonwoven gatherable web on the surface of the stretched nonwoven elastic web.

4. The process according to claims 1, 2 or 3, **characterized in that** the step of providing said nonwoven elastic web comprises forming a fibrous nonwoven elastic web of meltblown microfibers.

5. The process according to claims 1, 2 or 3, **characterized in that** the step of providing said nonwoven elastic web comprises providing an apertured elastic film.

6. The process according to claim 1, **characterized in that** the step of forming said fibrous nonwoven gatherable web comprises forming a fibrous nonwoven gatherable web of meltblow microfibers.

7. The process according to claims 1 or 2 and 4, **characterized in that** the step of forming said fibrous nonwoven gatherable web comprises forming a fibrous nonwoven gatherable web of spunbonded microfibers.

8. The process according to claim 1, **characterized in that** the step of forming said fibrous nonwoven gatherable web comprises forming a carded web.

9. The process according to claim 1, **characterized in that** the step of joining the fibrous nonwoven gatherable web to the nonwoven elastic web is achieved by heat-bonding.

10. The process according to claim 9, **characterized in that** the step of heat-bonding the fibrous nonwoven gatherable web to said nonwoven elastic web is achieved by heat-bonding within the temperature range of from about 50°C below a melting temperature of a material utilized to form either of the webs to about the melting temperature of a material utilized to form either of the webs.

11. The process according to claims 3 and 4, **characterized in that** said joining is achieved solely by entanglement of the individual fibers of the fibrous nonwoven gatherable web with the individual fibers of the fibrous nonwoven elastic web of meltblown microfibers.

12. The process according to claims 3 and 5, **characterized in that** said joining is achieved solely by entanglement of the individual fibers of the fibrous nonwoven gatherable web with the apertures of the apertured nonwoven elastic film.

13. The process according to any of claims 1 to 12 **characterized in that** the nonwoven elastic web comprises elastomeric fibers formed from a material selected from the group consisting essentially of A-B-A' block copolymers, wherein A and A' are each a thermoplastic polymer endblock comprising a styrenic moiety and where A may be the same thermoplastic endblock as A' and where B is an elastomeric polymer midblock selected from the group consisting of poly(ethylenebutylene), polyisoprene or polybutadiene.

14. The process according to any of claims 1 to 12, **characterized in that** the nonwoven elastic web comprises elastomeric fibers formed from a material selected from the group consisting essentially of blends of one or more polyolefins with S-EB-S block copolyers, where "S" is selected from the group consisting of polystyrene and polystyrene homologs and "EB" is poly (ethylenebutylene).

15. The process according to any of claims 1 to 12, **characterized in that** the nonwoven elastic web comprises elastomeric fibers formed from a material consisting essentially of blends of poly (alpha-methylstyrene) with S-I-S block copolymers, where "S" is selected from the group consisting of polystyrene and polystyrene homologs and "I" is polyisoprene.

16. The process according to claim 14, **characterized in that** the polyolefin is selected from the group consisting of at least one polymer, including copolymers, selected from the group consisting of ethylene, propylene and butene.

17. The process according to claim 16, **characterized in that** the polyolefin is polyethylene.

18. The process according to claim 6, **characterized in that** the fibrous nonwoven gatherable web comprises nonelastic meltblown microfibers.

19. The process according to claim 7, **characterized in that** the fibrous nonwoven gatherable web comprises nonelastic spunbonded microfibers.

20. The process according to claims 18 or 19, **characterized in that** the fibrous nonwoven gatherable web comprises nonelastic microfibers selected from the group consisting of polyester microfibers, polyolefin microfibers or blends of one or more polyester microfibers with one or more polyolefin microfibers.

21. The process according to claim 20, **characterized in that** the polyester microfibers comprise polyethylene terephthalate microfibers.

22. The process according to claim 20, **characterized in that** the polyolefin microfibers comprising the fibrous nonwoven gathered web comprise polypropylene microfibers.

23. The process according to claim 2, **characterized in that** the tacky fibrous nonwoven elastic web comprises tacky meltblown elastomeric microfibers formed from a material selected from the group consisting essentially of (a) A-B-A' block copolymers, where "A" and "A'" are thermoplastic polymer endblocks selected from the group consisting of polystyrene or polystyrene homologs and B is an elastomeric polymer midblock consisting of polyisoprene.

24. The process according to claim 23, **characterized in that** A and A' are selected from the group consisting of polystyrene.

25. The process according to claim 23, **characterized in that** the step of forming said fibrous nonwoven gatherable web comprises forming a fibrous nonwoven gatherable web of meltblown microfibers on the surface of said fibrous nonwoven elastic web.

26. A process for producing a gathered nonwoven web having elastic characteristics, comprising the step of:
a) providing an extendable and contractable forming surface,
**characterized in that** it further comprises the steps of
b) extending the forming surface from at least about 125% to about 700% of its unextended length;
c) forming a fibrous nonwoven gatherable web directly upon the extended forming surface to separably join the fibrous nonwoven gatherable web to the extended forming surface;
d) contracting the forming surface to gather the fibrous nonwoven gatherable web; and
e) separating the gathered fibrous nonwoven gatherable web from the contracted forming surface.

27. The process according to claim 26, **characterized in that** the extensible and contractable forming surface is a nonwoven elastic web having a relaxed, unbiased and contracted length and a stretched, biased and extended length; and the fibrous nonwoven gatherable web is formed directly upon a surface of said nonwoven elastic web forming surface to separably join said fibrous nonwoven gatherable web to said surface of said nonwoven elastic web forming surface while maintaining said nonwoven elastic web forming surface at said stretched length whereby the separable joining of the fibrous nonwoven gatherable web to the nonwoven elastic web forming surface is achieved by entanglement of the individual fibers of the nonwoven gatherable web with the individual fibers of the fibrous nonwoven elastic web forming surface during formation of the fibrous nonwoven gatherable web on the surface of the nonwoven elastic web forming surface.

28. The process according to claim 27, **characterized in that** the step of providing said nonwoven elastic web forming surface comprises forming a nonwoven elastic web of meltblown microfibers.

29. The process according to claim 26, **characterized in that** the step of forming said fibrous nonwoven gatherable web comprises forming a fibrous nonwoven gatherable web of spunbonded microfibers.

30. The process according to claim 26, **characterized in that** the step of forming said fibrous nonwoven gatherable web comprises forming a fibrous nonwoven gatherable web of spunbonded microfibers.

31. The process according to any of claims 26 to 30, **characterized in that** the gathered fibrous nonwoven web comprises nonelastic microfibers.

32. The process according to claim 31, **characterized in that** the gathered nonwoven elastic web comprises nonelastic meltblown microfibers selected from the group consisting of nonelastic poylester microfibers, nonelastic polyolefin microfibers or blends of one or more nonelastic polyester microfibers with one or more nonelastic polyolefin microfibers.

33. The process according to claim 31 **characterized in that** the gathered nonwoven elastic consists essentially of nonelastic spunbonded microfibers.

## Patentansprüche

1. Verfahren zur Herstellung eines nicht-gewebten, elastischen Verbundgewebes, umfassend ein nicht-gewebtes, elastisches Gewebe, das mit einem faserigen, nicht-gewebten, gerafften Gewebe verbunden ist, welches die folgende Stufe umfaßt:
(a) Bereitstellen eines nicht-gewebten, elastischen Gewebes,
**dadurch gekennzeichnet,** daß es weiterhin die folgenden Stufen umfaßt:
(b) Dehnen des nicht-gewebten, elastischen Gewebes von mindestens etwa 125 % der entspannten Länge des nicht-gewebten, elastischen Gewebes bis etwa 700 % der entspannten Länge des nicht-gewebten, elastischen Gewebes;
(c) Bilden eines faserigen, nicht-gewebten, raffbaren Gewebes direkt auf einer Oberfläche des gedehnten, nicht-gewebten, elastischen Gewebes und Verbinden des gedehnten, faserigen, nicht-gewebten, raffbaren Gewebes mit dem gedehnten, nicht-gewebten, elastischen Gewebe, um ein nicht-gewebtes, elastisches Verbundgewebe zu bilden; und
(d) Entspannen des nicht-gewebten, elastischen Verbundgewebes, um das faserige nicht-gewebte, raffbare Gewebe zu raffen.

2. Verfahren nach Anspruch 1, **dadurch gekennzeichnet,** daß das nicht-gewebte, elastische Gewebe ein klebendes, nicht-gewebtes, elastisches Gewebe ist und das nicht-gewebte, elastische Verbundgewebe durch Bilden eines faserigen, nicht-gewebten, raffbaren Gewebes direkt auf einer Oberfläche des gedehnten, nicht-gewebten, elastischen Gewebes und gleichzeitiges Verbinden des nicht-gewebten, elastischen Gewebes mit der Oberfläche des gedehnten, nicht-gewebten, elastischen Gewebes gebildet wird, wobei das Verbinden des klebrigen, nicht-gewebten, elastischen Gewebes mit dem faserigen nicht-gewebten, raffbaren Gewebe durch Adhaesion der beiden Gewebe aneinander während der Bildung des faserigen nicht-gewebten, raffbaren Gewebes auf der Oberfläche des gedehnten, faserigen, nicht-gewebten, elastischen Gewebes erzielt wird.

3. Verfahren nach Anspruch 1, **dadurch gekennzeichnet,** daß das nicht-gewebte, elastische Verbundgewebe durch Bilden eines faserigen, nicht-gewebten, raffbaren Gewebes direkt auf einer Oberfläche des gedehnten, nicht-gewebten, elastischen Gewebes und gleichzeitiges Verbinden des faserigen, nicht-gewebten, raffbaren Gewebes mit der Oberfläche des gedehnten, nicht-gewebten, elastischen Gewebes gebildet wird, wobei das Verbinden des nicht-gewebten, elastischen Gewebes mit dem faserigen, nicht-gewebten, raffbaren Gewebe durch Verhaken der einzelnen Fasern des faserigen, nicht-gewebten, raffbaren Gewebes mit dem nicht-gewebten, elastischen Gewebe während der Herstellung des faserigen, nicht-gewebten, raffbaren Gewebes auf der Oberfläche des gedehnten, nicht-gewebten, elastischen Gewebes erzielt wird.

4. Verfahren nach Anspruch 1, 2, oder 3, **dadurch gekennzeichnet,** daß die Stufe des Bereitstellens des nicht-gewebten, elastischen Gewebes das Bilden eines faserigen, nicht-gewebten, elastischen Gewebes aus schmelzgeblasenen Mikrofasern umfaßt.

5. Verfahren nach Anspruch 1, 2 oder 3, **dadurch gekennzeichnet,** daß die Stufe des Bereitstellens des nicht-gewebten, elastischen Gewebes das Bereitstellen eines löcherigen, elastischen Films umfaßt.

6. Verfahren nach Anspruch 1, **dadurch gekennzeichnet,** daß die Stufe des Bildens des faserigen, nicht-gewebten, raffbaren Gewebes das Bilden eines faserigen, nicht-gewebten, raffbaren Gewebes auf schmelzgeblasenen Mikrofasern umfaßt.

7. Verfahren nach Anspruch 1 oder 2 und 4, **dadurch gekennzeichnet,** daß die Stufe des Bildens des faserigen, nicht-gewebten, raffbaren Gewebes das Bilden eines faserigen, nicht-gewebten, raffbaren Gewebes aus zusammengesponnenen Mikrofasern umfaßt.

8. Verfahren nach Anspruch 1, **dadurch gekennzeichnet,** daß die Stufe des Bildens des faserigen, nicht-gewebten, raffbaren Gewebes das Bilden eines kardierten Gewebes umfaßt.

9. Verfahren nach Anspruch 1, **dadurch gekennzeichnet,** daß die Stufe des Verbindens des faserigen, nicht-gewebten, raffbaren Gewebes mit dem nicht-gewebten, elastischen Gewebe durch Wärmeverbinden erzielt wird.

10. Verfahren nach Anspruch 9, **dadurch gekennzeichnet,** daß die Stufe des Wärmeverbindes des faserigen, nicht-gewebten, raffbaren Gewebes mit dem nicht-gewebten, elastischen Gewebe durch Wärmeverbinden innerhalb eines Temperaturbereichs von etwa 50°C unter einer Schmelztemperatur eines Materials, das verwendet wird, um eines der Gewebe zu bilden, bis zu etwa der Schmelztemperatur eines Materials, das verwendet wird, um eines der Gewebe zu bilden, erzielt wird.

11. Verfahren nach Anspruch 3 und 4, **dadurch gekennzeichnet,** daß das Verbinden alleine durch Verhaken der einzelnen Fasern des faserigen, nicht-gewebten, raffbaren Gewebes mit den einzelnen Fasern des faserigen, nicht-gewebten, elastischen Gewebes aus schmelzgeblasenen Mikrofasern erzielt wird.

12. Verfahren nach Anspruch 3 und 5, **dadurch gekennzeichnet,** daß das Verbinden alleine durch Verhaken der einzelnen Fasern des faserigen, nicht-gewebten, raffbaren Gewebes mit den Löchern des löcherigen, nicht-gewebten, elastischen Films erzielt wird.

13. Verfahren nach einem der Ansprüche 1 bis 12, **dadurch gekennzeichnet,** daß das nicht-gewebte, elastische Gewebe Elastomerfasern, gebildet aus einem Material, ausgewählt aus der Gruppe, bestehend im wesentlichen aus A-B-A'-Blockcopolymeren, umfaßt, worin A und A' jeweils ein thermoplastischer Polymerendblock, umfassend einen Styrolteil sind, und worin A der gleiche thermoplastische Endblock wie A' sein kann und worin B ein elastomerer Polymermittelblock, ausgewählt aus der Gruppe, bestehend aus Poly(ethylenbutylen), Polyisopren oder Polybutadien, ist.

14. Verfahren nach einem der Ansprüche 1 bis 12, **dadurch gekennzeichnet,** daß das nicht-gewebte, elastische Gewebe Elastomerfasern, gebildet aus einem Material, ausgewählt aus der Gruppe, bestehend im wesentlichen aus Gemischen von einem oder mehreren Polyolefinen mit S-EB-S-Blockcopolymeren, umfaßt, worin "S" ausgewählt ist aus der Gruppe, bestehend aus Polystyrol und Polystyrol-homologen Verbindungen und "EB" Poly(ethylenbutylen) ist.

15. Verfahren nach einem der Ansprüche 1 bis 12, **dadurch gekennzeichnet,** daß das nicht-gewebte, elastische Gewebe Elastomerfasern, gebildet aus einem Material, bestehend im wesentlichen aus Gemischen von Poly(alpha-methylstyrol) mit S-I-S-Blockcopolymeren, umfaßt, worin "S" ausgewählt ist aus der Gruppe, bestehend aus Polystyrol und Polystyrol-homologen Verbindungen, und "I" Polyisopren ist.

16. Verfahren nach Anspruch 14, **dadurch gekennzeichnet,** daß das Polyolefin ausgewählt ist aus der Gruppe, bestehend aus mindestens einem Polymer, einschließlich Copolymeren, ausgewählt aus der Gruppe, bestehend aus Ethylen, Propylen und Buten.

17. Verfahren nach Anspruch 16, **dadurch gekennzeichnet,** daß das Polyolefin Polyethylen ist.

18. Verfahren nach Anspruch 6, **dadurch gekennzeichnet,** daß das faserige, nicht-gewebte, raffbare Gewebe unelastische schmelzgeblasene Mikrofasern umfaßt.

19. Verfahren nach Anspruch 7, **dadurch gekennzeichnet,** daß das faserige, nicht-gewebte, raffbare Gewebe unelastische, zusammengesponnene Mikrofasern umfaßt.

20. Verfahren nach Anspruch 18 oder 19, **dadurch gekennzeichnet,** daß das faserige, nicht-gewebte, raffbare Gewebe unelastische Mikrofasern, ausgewählt aus der Gruppe, bestehend aus Polyestermikrofasern, Polyolefinmikrofasern oder Gemischen von einem oder mehreren Polyestermikrofasern mit einer oder mehreren Polyolefinmikrofasern, umfaßt.

21. Verfahren nach Anspruch 20, **dadurch gekennzeichnet,** daß die Polyestermikrofasern Polyethylenterephthalatmikrofasern umfassen.

22. Verfahren nach Anspruch 20, **dadurch gekennzeichnet,** daß die Polyolefinmikrofasern, umfassend das faserige, nicht-gewebte, raffbare Gewebe, Polypropylenmikrofasern umfassen.

23. Verfahren nach Anspruch 2, **dadurch gekennzeichnet,** daß das klebrige, faserige, nicht-gewebte, elastische Gewebe klebrige, schmelzgeblasene elastomere Mikrofasern, gebildet aus einem Material, ausgewählt aus der Gruppe, bestehend im wesentlichen aus (a) A-B-A' Blockcopolymeren, umfaßt, worin "A" und "A'" thermoplastische Polymerendblöcke, ausgewählt aus der Gruppe, bestehend aus Polystyrol oder Polystyrol-homologen Verbindungen, sind und B ein elastomerer Polymermittelblock, bestehend aus Polyisopren, ist.

24. Verfahren nach Anspruch 23, **dadurch gekennzeichnet,** daß A und A' aus der Gruppe, bestehend aus Polystyrol, ausgewählt sind.

25. Verfahren nach Anspruch 23, **dadurch gekennzeichnet,** daß die Stufe des Bildens des faserigen, nicht-gewebten, raffbaren Gewebes das Bilden eines faserigen, nicht-gewebten, raffbaren Gewebes aus schmelzgeblasenen Mikrofasern auf der Oberfläche des faserigen, nicht-gewebten, raffbaren Gewebes umfaßt.

26. Verfahren zur Herstellung eines gerafften, nicht-gewebten Gewebes mit elastischen Eigenschaften, umfassend die folgende Stufe:
(a) Bereitstellen einer dehnbaren und zusammenziehbaren Formoberfläche
**dadurch gekennzeichnet,** daß es weiterhin die folgenden Stufen umfaßt:
(b) Dehnen der Formoberfläche von mindestens etwa 125 % bis etwa 700 % ihrer ungedehnten Länge;
(c) Bilden eines faserigen, nicht-gewebten, raffbaren Gewebes direkt auf der gedehnten Formoberfläche, um das faserige, nicht-gewebte, raffbare Gewebe abtrennbar mit der gedehnten Formoberfläche zu verbinden;
(d) Zusammenziehen der Formoberfläche, um das faserige, nicht-gewebte, raffbare Gewebe zu raffen; und
(e) Trennen des gerafften, faserigen, nicht-gewebten, raffbaren Gewebes von der zusammengezogenen Formoberfläche.

27. Verfahren nach Anspruch 26, **dadurch gekennzeichnet,** daß die dehnbare und zusammenziehbare Formoberfläche ein nicht-gewebtes, elastisches Gewebe mit einer entspannten, unregelmäßigen und zusammengezogenen Länge und einer gedehnten, regelmäßigen und verlängerten Länge ist; und das faserige, nicht-gewebte, raffbare Gewebe direkt auf einer Oberfläche der Formoberfläche aus dem nicht-gewebten, elastischen Gewebe gebildet wird, um das faserige, nicht-gewebte, raffbare Gewebe abtrennbar mit der Oberfläche der Formoberfläche aus dem nicht-gewebten, elastischen Gewebe zu verbinden, während die Formoberfläche aus dem nicht-gewebten, elastischen Gewebe in seiner gedehnten Länge gehalten wird, wobei das abtrennbare Verbinden des faserigen, nicht-gewebten, raffbaren Gewebes mit der Formoberfläche aus dem nicht-gewebten, elastischen Gewebe durch Verhaken der einzelnen Fasern des nicht-gewebten, raffbaren Gewebes mit den einzelnen Fasern der Formoberfläche aus dem faserigen, nicht-gewebten, elastischen Gewebe während der Herstellung des faserigen, nicht-gewebten, raffbaren Gewebes auf der Oberfläche der Formoberfläche aus dem nicht-gewebten, elastischen Gewebe erzielt wird.

28. Verfahren nach Anspruch 27, **dadurch gekennzeichnet,** daß die Stufe des Bereitstellens der Formoberfläche aus dem nicht-gewebten, elastischen Gewebe das Bilden eines nicht-gewebten, elastischen Gewebes aus schmelzgeblasenen Mikrofasern umfaßt.

29. Verfahren nach Anspruch 26, **dadurch gekennzeichnet,** daß die Stufe des Bildens des faserigen, nicht-gewebten, raffbaren Gewebes das Bilden eines faserigen, nicht-gewebten, raffbaren Gewebes aus zusammengesponnenen Mikrofasern umfaßt.

30. Verfahren nach Anspruch 26, **dadurch gekennzeichnet,** daß die Stufe des Bildens des faserigen, nicht-gewebten, raffbaren Gewebes das Bilden eines faserigen, nicht-gewebten, raffbaren Gewebes aus zusammengesponnenen Mikrofasern umfaßt.

31. Verfahren nach einem der Ansprüche 26 bis 30, **dadurch gekennzeichnet,** daß das geraffte, faserige, nicht-gewebte Gewebe unelastische Mikrofasern umfaßt.

32. Verfahren nach Anspruch 31, **dadurch gekennzeichnet,** daß das geraffte, nicht-gewebte, elastische Gewebe unelastische, schmelzgeblasene Mikrofasern, ausgewählt aus der Gruppe, bestehend aus unelastischen Polyestermikrofasern, unelastischen Polyolefinmikrofasern oder Gemischen aus einer oder mehreren unelastischen Polyestermikrofasern mit einer oder mehreren unelastischen Polyolefinmikrofasern, umfaßt.

33. Verfahren nach Anspruch 31, **dadurch gekennzeichnet,** daß das geraffte, nicht-gewebte, elastische Gewebe im wesentlichen aus unelastischen zusammengesponnenen Mikrofasern besteht.

## Revendications

1. Procédé de fabrication d'une étoffe élastique non tissée composite, comportant une étoffe élastique non tissée jointe à une étoffe froncée non tissée fibreuse, comprenant l'étape qui consiste :
(a) à disposer d'une étoffe élastique non tissée,
caractérisé par les étapes ultérieures qui consistent :
(b) à étirer ladite étoffe élastique non tissée depuis au moins environ 125% de la longueur détendue de l'étoffe élastique non tissée jusqu'à environ 700% de la longueur détendue de l'étoffe élastique non tissée ;
(c) à former une étoffe non tissée fibreuse pouvant être froncée directement au-dessus de la surface de l'étoffe élastique non tissée étirée, et à joindre l'étoffe non tissée fibreuse étirée pouvant être froncée à l'étoffe élastique non tissée étirée de manière à former une étoffe élastique non tissée composite ; et
(d) à relâcher l'étoffe élastique non tissée composite pour froncer l'étoffe non tissée fibreuse pouvant être froncée.

2. Procédé selon la revendication 1, caractérisé en ce que l'étoffe élastique non tissée est une étoffe élastique non tissée collante et l'étoffe élastique non tissée composite est constituée par formage d'une étoffe non tissée fibreuse pouvant être froncée directement au-dessus d'une surface de l'étoffe élastique non tissée étirée_{,} et en joignant simultanément ladite étoffe élastique non tissée à la surface de l'étoffe élastique non tissée étirée, ce par quoi la liaison de l'étoffe élastique non tissée collante à l'étoffe non tissée fibreuse pouvant être froncée est réalisée par adhérence des deux étoffes l'une à l'autre au cours de la formation de l'étoffe non tissée fibreuse pouvant être froncée sur la surface de l'étoffe élastique non tissée fibreuse étirée.

3. Procédé selon la revendication 1, caractérisé en ce que l'étoffe élastique non tissée composite est constituée par formage d'une étoffe non tissée fibreuse pouvant être froncée directement au-dessus d'une surface d'une étoffe élastique non tissée étirée, et en joignant simultanément l'étoffe non tissée fibreuse pouvant être froncée à la surface de l'étoffe élastique non tissée étirée, par laquelle la liason de l'étoffe élastique non tissée à l'étoffe non tissée fibreuse pouvant être froncée est réalisée par l'enchevêtrement des fibres individuelles de l'étoffe non tissée fibreuse pouvant être froncée avec l'étoffe élastique non tissée au cours du formage de l'étoffe non tissés fibreuse pouvant être froncée sur la surface de l'étoffe élastique non tissée étirée.

4. Procédé selon les revendications 1, 2 ou 3, caractérisé en ce que l'étape qui consiste à disposer ladite étoffe élastique non tissée comporte le formage d'une étoffe élastique non tissée fibreuse des microfibres obtenues par soufflage par fusion.

5. Procédé selon les revendications 1, 2 ou 3, caractérisé en ce que l'étape qui consiste à disposer de ladite étoffe élastique non tissée consiste à disposer d'un film élastique fendu.

6. Procédé selon la revendication 1, caractérise en ce que l'étape de formage de ladite étoffe non tissée fibreuse pouvant être froncée comporte la formage d'une étoffe non tissée fibreuse pouvant être froncée de microfibres obtenues par soufflage par fusion.

7. Procédé selon les revendications 1 ou 2 et 4, caractérisé en ce que l'étape de formage de ladite étoffe non tissée fibreuse pouvant être froncée comporte le formage d'une étoffe non tissée fibreuse pouvant être froncée de microfibres assemblées par filage.

8. Procédé selon la revendication 1, caractérisé en ce que l'étape de formage de ladite étoffe non tissée fibreuse pouvant être froncée comporte le formage d'une étoffe cardée.

9. Procédé selon la revendication 1, caractérisé en ce que l'étape de liason de l'étoffe non tissée fibreuse pouvant être froncée à l'étoffe élastique non tissée est réalisée par assemblage thermique.

10. Procédé selon la revendication 9, caractérisé en ce que l'étape d'assemblage thermique de l'étoffe non tissée fibreuse pouvant être froncée à ladite étoffe élastique non tissée est réalisée par assemblage thermique dans un intervalle de température compris entre environ 50 degrés Celsius au-dessous de la température de fusion d'un matériau utilisé pour l'une ou l'autre des étoffes, jusqu'à environ la température de fusion d'un matériau utilisé pour former l'une ou l'autre des étoffes.

11. Procédé selon les revendications 3 et 4, caractérisé en ce que ladite liason est réalisée uniquement par l'enchevêtrement de fibres individuelles de l'étoffe non tissée fibreuse pouvant être froncée avec les fibres individuelles de l'étoffe élastique non tissée fibreuse de microfibres soufflées par soufflage par fusion.

12. Procédé selon les revendications 3 et 5, caractérisé en ce que ladite liason est réalisée uniquement par l'enchevêtrement de fibres individuelles de l'étoffe non tissée fibreuse pouvant être froncée dans les fentes du film élastique non tissé fendu.

13. Procédé selon l'une quelconque des revendications 1 à 12, caractérisé en ce que l'étoffe élastique non tissée comporte des fibres élastomères formées par un matériau sélectionné à partir du groupe constitué essentiellement par des copolymères de blocs A-B-A', dans lesquels A et A' sont chacun un bloc d'extrémité de polymères thermoplastiques comportant une demi-portion de styrène et où A peut être le même bloc d'extrémité thermoplastique que A' et où B est un bloc médian de polymères élastomères sélectionnés à partir du groupe constitué par du poly(éthylènebutylène), du poly-isoprène ou du polybutadiène.

14. Procédé selon l'une quelconque des revendications 1 à 12, caractérisé en ce que l'étoffe élastique non tissée comporte des fibres élastomères formées par un matériau sélectionné à partir du groupe constitué essentiellement de mélanges d'un ou plusieurs polyoléfines avec des copolymères de blocs S-EB-S, où "S" est sélectionné à partir du groupe constitué par du polystyrène et des homologues du poltstyrène, et où "EB" est constitué par du poly(éthylènebutylène).

15. Procédé selon l'une quelconque des revendications 1 à 12, caractérisé en ce que l'étoffe élastique non tissée comporte des fibres élastomères formées à partir d'un matériau constitué essentiellement par des mélanges de poly(alpha-méthylstyrène) et de copolymères en blocs S-I-S, où "S" est sélectionné à partir du groupe constitué par du polystyrène et des homologues de polystyrène, et "I" est du poly-isoprène.

16. Procédé selon la revendication 14, caractérisé en ce que le polyoléfine est sélectionné à partir du groupe constitué par au moins un polymère comprenant des copolymères sélectionnés à partir du groupe constitué par de l'éthylène, du propylène et du butène.

17. Procédé selon la revendication 16, caractérisé en ce que le polyoléfine est du polyéthylène.

18. Procédé selon la revendication 6, caractérisé en ce que l'étoffe non tissée fibreuse pouvant être froncée comporte des microfibres non élastiques obtenues par soufflage par fusion.

19. Procédé selon la revendication 7, caractérisé en ce que l'étoffe non tissée fibreuse pouvant être froncée comporte des microfibres non élastiques assemblées par filage.

20. Procédé selon les revendications 18 ou 19, caractérisé en ce que l'étoffe non tissée fibreuse pouvant être froncée comporte des microfibres non élastiques sélectionnées à partir du groupe constitué par des microfibres de polyester, des microfibres de polyoléfines ou des mélanges d'une ou plusieurs microfibres de polyester avec une ou plusieurs microfibres de polyoléfine.

21. Procédé selon la revendication 20, caractérisé en ce que les microfibres de polyester comportent des microfibres en téréphtalate de polyéthylène.

22. Procédé selon la revendication 20, caractérisé en ce que les microfibres de polyoléfine comportant une étoffe non tissée fibreuse froncée comprend des microfibres de polypropylène.

23. Procédé selon la revendication 2, caractérise en ce que l'étoffe élastique non tissée fibreuse collante comporte des microfibres élastomères collantes obtenues par soufflage par fusion formées par un matériau sélectionné à partir du groupe constitué essentiellement par (a) des copolymères en blocs A-B-A', dans lesquels "A" et "A'" sont des blocs d'extrémité de polymères thermoplastiques sélectionnés à partir du groupe constitué par du polystyrène ou des homologues du polystyrène et B est un bloc médian d'un polymère élastomère constitué par du poly-isoprène.

24. Procédé selon la revendication 23, caractérisé en ce que A et A' sont sélectionnés à partir du groupe constitué par du polystyrène.

25. Procédé selon la revendication 23, caractérisé en ce que l'étape de formage de ladite étoffe non tissée fibreuse pouvant être froncée comporte le formage d'une étoffe non tissée fibreuse pouvant être froncée de microfibres obtenues par soufflage par fusion sur la surface de ladite étoffe élastique non tissée fibreuse.

26. Procédé de fabrication d'une étoffe non tissée froncée ayant des caractéristiques élastiques, comportant l'étape qui consiste :
(a) à disposer d'une surface de formage extensible et contractile,
caractérisé en ce qu'il comporte les étapes ultérieures qui consistent :
(b) à allonger la surface de formage depuis au moins environ 125% jusqu'à environ 700% de sa longueur non allongée ;
(c) à former une étoffe non tissée fibreuse pouvant être froncée directement au-dessus de la surface de formage allongée pour joindre de façon séparable l'étoffe non tissée fibreuse pouvant être froncée à la surface de formage allongée ;
(d) à contracter la surface de formage pour froncer l'étoffe non tissée pouvant être froncée ; et
(e) à séparer l'étoffe non tissée fibreuse pouvant être froncée qui est ainsi froncée, de la surface de formage contractée.

27. Procédé selon la revendication 26, caractérisé en ce que la surface de formage extensible et contractile est une étoffe élastique non tissée ayant une longueur détendue sans contrainte et contractée et une longueur étirée soumise à des contraintes et allongée ; l'étoffe non tissée fibreuse pouvant être froncée étant formée directement au-dessus de ladite surface de formage élastique non tissée pour joindre de façon séparable ladite étoffe non tissée fibreuse pouvant être froncée à ladite surface de formage de ladite étoffe élastique non tissée, tout en maintenant ladite surface de formage de l'étoffe élastique non tissée suivant ladite longueur étirée, ce par quoi la liason séparable de l'étoffe non tissée fibreuse pouvant être froncée à ladite surface de formage de l'étoffe élastique non tissée est réalisée par l'enchevêtrement des fibres individuelles de l'étoffe non tissée pouvant être froncée avec les fibres individuelles de la surface de formage de l'étoffe élastique non tissée fibreuse au cours du formage de l'étoffe non tissée fibreuse pouvant être froncée sur la surface de formage de l'étoffe élastique non tissée.

28. Procédé selon la revendication 27, caractérisé en ce que l'étape qui consiste à disposer de ladite surface de formage de l'étoffe élastique non tissée comporte le formage d'une étoffe élastique non tissée de microfibres obtenues par soufflage par fusion.

29. Procédé selon la revendications 26, caractérisé en ce que l'étape de formage de ladite étoffe non tissée fibreuse pouvant être froncée comporte le formage d'une surface non tissée fibreuse pouvant être froncée de microfibres assemblées par filage.

30. Procédé selon la revendication 26, caractérisé en ce que l'étape de formage de ladite étoffe non tissée fibreuse pouvant être froncée comporte le formage d'une étoffe non tissée fibreuse pouvant être froncée constituée par des microfibres assemblées par filage.

31. Procédé selon l'une quelconque des revendications 26 à 30, caractérisé en ce que l'étoffe non tissée fibreuse froncée comporte des microfibres non élastiques.

32. Procédé selon la revendication 31, caractérisé en ce que l'étoffe élastique non tissée froncée comporte des microfibres non élastiques obtenues par soufflage par fusion sélectionnées à partir du groupe constitué par des microfibres en polyester non élastique, des microfibres en polyoléfine non élastique ou en des mélanges d'une ou plusieurs microfibres en polyester non élastique avec une ou plusieurs microfibres en polyoléfine non élastique.

33. Procédé selon la revendication 31, caractérisé en ce que l'étoffe élastique non tissée froncée consiste essentiellement en microfibres non élastiques assemblées par filage.
